



US006260956B1

(12) **United States Patent**  
Narang et al.

(10) **Patent No.:** US 6,260,956 B1  
(45) **Date of Patent:** Jul. 17, 2001

- (54) **THERMAL INK JET PRINthead AND PROCESS FOR THE PREPARATION THEREOF**
- (75) Inventors: **Ram S. Narang**, Fairport; **Gary A. Knezel**, Webster; **Bidan Zhang**, Beacon; **Almon P. Fisher**, Rochester; **Timothy J. Fuller**, Pittsford, all of NY (US)
- (73) Assignee: **Xerox Corporation**, Stamford, CT (US)
- (\*) Notice: Subject to any disclaimer, the term of this patent is extended or adjusted under 35 U.S.C. 154(b) by 0 days.
- (21) Appl. No.: **09/120,746**
- (22) Filed: **Jul. 23, 1998**
- (51) **Int. Cl.**<sup>7</sup> ..... **B41J 2/04**; B41J 2/015; G01D 15/16; G11B 5/127
- (52) **U.S. Cl.** ..... **347/63**; 347/64; 347/65; 347/20; 347/54; 216/27; 156/145; 427/504
- (58) **Field of Search** ..... 347/20, 40, 47, 347/54, 60; 427/504; 216/27; 522/162, 163, 164, 166; 430/270.1, 280.1, 281.1; 156/145

(56) **References Cited**

U.S. PATENT DOCUMENTS

- 4,739,032 4/1988 Jones ..... 528/230  
5,738,799 4/1998 Hawkins et al. ..... 216/27  
5,739,254 4/1998 Fuller et al. ..... 528/125  
5,753,783 5/1998 Fuller et al. ..... 525/471  
5,761,809 6/1998 Fuller et al. ..... 29/890.1  
5,849,809 \* 12/1998 Narang et al. ....  
5,863,963 \* 1/1999 Narang et al. ....  
5,889,077 \* 3/1999 Fuller et al. ....  
5,945,253 \* 8/1999 Narang et al. ....

- 5,958,995 \* 9/1999 Narang et al. ....  
5,994,425 \* 11/1999 Narang et al. ....  
6,007,877 \* 12/1999 Narang et al. ....  
6,090,453 \* 7/2000 Narang et al. ....  
6,124,372 \* 9/2000 Smith et al. ....  
6,151,042 \* 11/2000 Smith et al. ....

FOREIGN PATENT DOCUMENTS

- 0 827 027 A2 3/1998 (EP) ....  
0 827 028 A2 3/1998 (EP) ....  
0 827 029 A2 3/1998 (EP) ....  
0 827 030 A2 3/1998 (EP) ....  
0 827 031 A2 3/1998 (EP) ....  
0 827 032 A2 3/1998 (EP) ....  
0 827 033 A2 3/1998 (EP) ....

\* cited by examiner

Primary Examiner—Susan W. Berman

(74) Attorney, Agent, or Firm—Judith L. Byorick

(57) **ABSTRACT**

Disclosed is an ink jet printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the printhead with the grooves in the upper substrate being aligned with the heating elements in the lower substrate to form droplet emitting nozzles, said upper substrate comprising a material formed by crosslinking or chain extending a polymer of formula I or II.

**20 Claims, 3 Drawing Sheets**





FIG. 1



FIG. 2



### FIG. 3

**THERMAL INK JET PRINthead AND  
PROCESS FOR THE PREPARATION  
THEREOF**

**BACKGROUND OF THE INVENTION**

The present invention is directed to thermal ink jet printheads. More specifically, the present invention is directed to thermal ink jet printheads wherein the upper or channel plate thereof is formed of a specific polymeric material. In some embodiments, the insulative layer of the lower or heater plate of the printhead is formed of this polymeric material. In other embodiments, the lower and upper plates of the printhead are bonded together by an adhesive which comprises this polymeric material. In still other embodiments, the printhead is substantially free of an interface between the lower substrate and the upper substrate. One embodiment of the present invention is directed to an ink jet printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the printhead with the grooves in the upper substrate being aligned with the heating elements in the lower substrate to form droplet emitting nozzles, said upper substrate comprising a material formed by crosslinking or chain extending a polymer of the formula

each integers of 0, 1, 2, 3, or 4, provided that at least one of a, b, c, and d is equal to or greater than 1 in at least some of the monomer repeat units of the polymer, A is



35

I



or



or mixtures thereof, B is



wherein x is an integer of 0 or 1, P is a substituent which imparts photosensitivity to the polymer, a, b, c, and d are

3

-continued



4

-continued



wherein v is an integer of from 1 to about 20, and preferably from 1 to about 10,



wherein z is an integer of from 2 to about 20, and preferably from 2 to about 10,



wherein u is an integer of from 1 to about 20, and preferably from 1 to about 10,



or mixtures thereof, and n is an integer representing the number of repeating monomer units.

Ink jet printing systems generally are of two types: 50 continuous stream and drop-on-demand. In continuous stream ink jet systems, ink is emitted in a continuous stream under pressure through at least one orifice or nozzle. The stream is perturbed, causing it to break up into droplets at a fixed distance from the orifice. At the break-up point, the 55 droplets are charged in accordance with digital data signals and passed through an electrostatic field which adjusts the trajectory of each droplet in order to direct it to a gutter for recirculation or a specific location on a recording medium. In drop-on-demand systems, a droplet is expelled from an 60 orifice directly to a position on a recording medium in accordance with digital data signals. A droplet is not formed or expelled unless it is to be placed on the recording medium.

Since drop-on-demand systems require no ink recovery, 65 charging, or deflection, the system is much simpler than the continuous stream type. There are different types of drop-on-demand ink jet systems. One type of drop-on-demand

system has as its major components an ink filled channel or passageway having a nozzle on one end and a piezoelectric transducer near the other end to produce pressure pulses. The relatively large size of the transducer prevents close spacing of the nozzles, and physical limitations of the transducer result in low ink drop velocity. Low drop velocity seriously diminishes tolerances for drop velocity variation and directionality, thus impacting the system's ability to produce high quality copies. Drop-on-demand systems which use piezoelectric devices to expel the droplets also suffer the disadvantage of a slow printing speed.

Another type of drop-on-demand system is known as thermal ink jet, or bubble jet, and produces high velocity droplets and allows very close spacing of nozzles. The major components of this type of drop-on-demand system are an ink filled channel having a nozzle on one end and a heat generating resistor near the nozzle. Printing signals representing digital information originate an electric current pulse in a resistive layer within each ink passageway near the orifice or nozzle, causing the ink in the immediate vicinity to vaporize almost instantaneously and create a bubble. The ink at the orifice is forced out as a propelled droplet as the bubble expands. When the hydrodynamic motion of the ink stops, the process is ready to start all over again. With the introduction of a droplet ejection system based upon thermally generated bubbles, commonly referred to as the "bubble jet" system, the drop-on-demand ink jet printers provide simpler, lower cost devices than their continuous stream counterparts, and yet have substantially the same high speed printing capability.

The operating sequence of the bubble jet system begins with a current pulse through the resistive layer in the ink filled channel, the resistive layer being in close proximity to the orifice or nozzle for that channel. Heat is transferred from the resistor to the ink. The ink becomes superheated far above its normal boiling point, and for water based ink, finally reaches the critical temperature for bubble formation or nucleation of around 280° C. Once nucleated, the bubble or water vapor thermally isolates the ink from the heater and no further heat can be applied to the ink. This bubble expands until all the heat stored in the ink in excess of the normal boiling point diffuses away or is used to convert liquid to vapor, which removes heat due to heat of vaporization. The expansion of the bubble forces a droplet of ink out of the nozzle, and once the excess heat is removed, the bubble collapses. At this point, the resistor is no longer being heated because the current pulse has passed and, concurrently with the bubble collapse, the droplet is propelled at a high rate of speed in a direction towards a recording medium. The surface of the printhead encounters a severe cavitation force by the collapse of the bubble, which tends to erode it. Subsequently, the ink channel refills by capillary action. This entire bubble formation and collapse sequence occurs in about 10 microseconds. The channel can be refired after 100 to 500 microseconds minimum dwell time to enable the channel to be refilled and to enable the dynamic refilling factors to become somewhat damped. Thermal ink jet equipment and processes are well known and are described in, for example, U.S. Pat. Nos. 4,601,777, 4,251,824, 4,410,899, 4,412,224, 4,532,530, and 4,774,530, the disclosures of each of which are totally incorporated herein by reference.

In ink jet printing, a printhead is usually provided having one or more ink-filled channels communicating with an ink supply chamber at one end and having an opening at the opposite end, referred to as a nozzle. These prinheads form images on a recording medium such as paper by expelling

droplets of ink from the nozzles onto the recording medium. The ink forms a meniscus at each nozzle prior to being expelled in the form of a droplet. After a droplet is expelled, additional ink surges to the nozzle to reform the meniscus.

In thermal ink jet printing, a thermal energy generator, usually a resistor, is located in the channels near the nozzles a predetermined distance therefrom. The resistors are individually addressed with a current pulse to momentarily vaporize the ink and form a bubble which expels an ink droplet. As the bubble grows, the ink bulges from the nozzle and is contained by the surface tension of the ink as a meniscus. The rapidly expanding vapor bubble pushes the column of ink filling the channel towards the nozzle. At the end of the current pulse the heater rapidly cools and the vapor bubble begins to collapse. However, because of inertia, most of the column of ink that received an impulse from the exploding bubble continues its forward motion and is ejected from the nozzle as an ink drop. As the bubble begins to collapse, the ink still in the channel between the nozzle and bubble starts to move towards the collapsing bubble, causing a volumetric contraction of the ink at the nozzle and resulting in the separation of the bulging ink as a droplet. The acceleration of the ink out of the nozzle while the bubble is growing provides the momentum and velocity of the droplet in a substantially straight line direction towards a recording medium, such as paper.

Ink jet printheads include an array of nozzles and have commonly been formed of silicon wafers using orientation dependent etching (ODE) techniques. The resulting nozzles are generally triangular in cross-section. Thermal ink jet printheads made by using the above-mentioned ODE techniques typically comprise a channel plate which contains a plurality of nozzle-defining channels located on a lower surface thereof bonded to a heater plate having a plurality of resistive heater elements formed on an upper surface thereof and arranged so that a heater element is located in each channel. The upper surface of the heater plate typically includes an insulative layer which is patterned to form recesses exposing the individual heating elements. This insulative layer is referred to as a "pit layer" and is sandwiched between the channel plate and heater plate. For examples of printheads employing this construction, see U.S. Pat. Nos. 4,774,530 and 4,829,324, the disclosures of each of which are totally incorporated herein by reference. Additional examples of thermal ink jet printheads are disclosed in, for example, U.S. Pat. Nos. 4,835,553, 5,057,853, and 4,678,529, the disclosures of each of which are totally incorporated herein by reference.

U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas W. Smith, David J. Luca, and Raymond K. Crandall, and European Patent Publication 0,826,700, the disclosures of each of which are totally incorporated herein by reference, disclose a process which comprises reacting a polymer of the general formula



or



wherein x is an integer of 0 or 1, A is one of several specified groups, such as



B is one of several specified groups, such as



or mixtures thereof, and n is an integer representing the number of repeating monomer units, with an acetyl halide and dimethoxymethane in the presence of a halogen-containing Lewis acid catalyst and methanol, thereby forming a haloalkylated polymer. In a specific embodiment, the haloalkylated polymer is then reacted further to replace at least some of the haloalkyl groups with photosensitivity-imparting groups. Also disclosed is a process for preparing a thermal ink jet printhead with the aforementioned polymer.

U.S. Pat. No. 5,761,809, filed Aug. 29, 1996, entitled "Processes for Substituting Haloalkylated Polymers With Unsaturated Ester, Ether, and Alkylcarboxymethylene Groups," with the named inventors Timothy J. Fuller, Ram S. Narang, Thomas W. Smith, David J. Luca, and Raymond K. Crandall, and European Patent Publication 0,827,026, the disclosures of each of which are totally incorporated herein by reference, disclose a process which comprises reacting a haloalkylated aromatic polymer with a material selected from the group consisting of unsaturated ester salts, alkoxide salts, alkylcarboxylate salts, and mixtures thereof, thereby forming a curable polymer having functional groups corresponding to the selected salt. Another embodiment of the

invention is directed to a process for preparing an ink jet printhead with the curable polymer thus prepared.

U.S. Pat. No. 5,738,799, filed Sep. 12, 1996, the disclosure of which is totally incorporated herein by reference, discloses an ink-jet printhead fabrication technique which enables capillary channels for liquid ink to be formed with square or rectangular cross-sections. A sacrificial layer is placed over the main surface of a silicon chip, the sacrificial layer being patterned in the form of the void formed by the desired ink channels. A permanent layer, comprising permanent material, is applied over the sacrificial layer, and, after polishing the two layers to form a uniform surface, the sacrificial layer is removed. Preferred materials for the sacrificial layer include polyimide while preferred materials for the permanent layer include polyarylene ether, although a variety of material combinations are possible.

Copending application U.S. Ser. No. 08/705,914, filed Aug. 29, 1996, entitled "Thermal Ink Jet Printhead With Ink Resistant Heat Sink Coating," with the named inventors Ram S. Narang and Timothy J. Fuller, the disclosure of which is totally incorporated herein by reference, discloses a heat sink for a thermal ink jet printhead having improved resistance to the corrosive effects of ink by coating the surface of the heat sink with an ink resistant film formed by electrophoretically depositing a polymeric material on the heat sink surface. In one described embodiment, a thermal ink jet printer is formed by bonding together a channel plate and a heater plate. Resistors and electrical connections are formed in the surface of the heater plate. The heater plate is bonded to a heat sink comprising a zinc substrate having an electrophoretically deposited polymeric film coating. The film coating provides resistance to the corrosion of higher pH inks. In another embodiment, the coating has conductive fillers dispersed therethrough to enhance the thermal conductivity of the heat sink. In one embodiment, the polymeric material is selected from the group consisting of polyethersulfones, polysulfones, polyamides, polyimides, polyamide-imides, epoxy resins, polyetherimides, polyarylene ether ketones, chloromethylated polyarylene ether ketones, acryloylated polyarylene ether ketones, polystyrene and mixtures thereof.

Copending application U.S. Ser. No. 08/703,138, filed Aug. 29, 1996, entitled "Method for Applying an Adhesive Layer to a Substrate Surface," with the named inventors Ram S. Narang, Stephen F. Pond, and Timothy J. Fuller, the disclosure of which is totally incorporated herein by reference, discloses a method for uniformly coating portions of the surface of a substrate which is to be bonded to another substrate. In a described embodiment, the two substrates are channel plates and heater plates which, when bonded together, form a thermal ink jet printhead. The adhesive layer is electrophoretically deposited over a conductive pattern which has been formed on the binding substrate surface. The conductive pattern forms an electrode and is placed in an electrophoretic bath comprising a colloidal emulsion of a preselected polymer adhesive. The other electrode is a metal container in which the solution is placed or a conductive mesh placed within the container. The electrodes are connected across a voltage source and a field is applied. The substrate is placed in contact with the solution, and a small current flow is carefully controlled to create an extremely uniform thin deposition of charged adhesive micelles on the surface of the conductive pattern. The substrate is then removed and can be bonded to a second substrate and cured. In one embodiment, the polymer adhesive is selected from the group consisting of polyamides, polyimides, polyamide-imides, epoxy resins,

polyetherimides, polysulfones, polyether sulfones, polyarylene ether ketones, polystyrenes, chloromethylated polyarylene ether ketones, acryloylated polyarylene ether ketones, and mixtures thereof.

Copending application U.S. Ser. No. 08/697,750, filed Aug. 29, 1996, entitled "Electrophoretically Deposited Coating For the Front Face of an Ink Jet Printhead," with the named inventors Ram S. Narang, Stephen F. Pond, and Timothy J. Fuller, the disclosure of which is totally incorporated herein by reference, discloses an electrophoretic deposition technique for improving the hydrophobicity of a metal surface, in one embodiment, the front face of a thermal ink jet printhead. For this example, a thin metal layer is first deposited on the front face. The front face is then lowered into a colloidal bath formed by a fluorocarbon-doped organic system dissolved in a solvent and then dispersed in a non-solvent. An electric field is created and a small amount of current through the bath causes negatively charged particles to be deposited on the surface of the metal coating. By controlling the deposition time and current strength, a very uniform coating of the fluorocarbon compound is formed on the metal coating. The electrophoretic coating process is conducted at room temperature and enables a precisely controlled deposition which is limited only to the front face without intrusion into the front face orifices. In one embodiment, the organic compound is selected from the group consisting of polyimides, polyamides, polyamide-imides, polysulfones, polyarylene ether ketones, polyethersulfones, polytetrafluoroethylenes, polyvinylidene fluorides, polyhexafluoro-propylenes, epoxies, polyperfluorostyrenes, polystyrenes, copolymers thereof, terpolymers thereof, and mixtures thereof.

Copending application U.S. Ser. No. 08/705,916, filed Aug. 29, 1996, entitled "Stabilized Graphite Substrates," with the named inventors Gary A. Kneezel, Ram S. Narang, Timothy J. Fuller, and Peter J. John, the disclosure of which is totally incorporated herein by reference, discloses an apparatus which comprises at least one semiconductor chip mounted on a substrate, said substrate comprising a graphite member having electrophoretically deposited thereon a coating of a polymeric material. In one embodiment, the semiconductor chips are thermal ink jet printhead subunits. In one embodiment, the polymeric material is of the general formula



or



wherein x is an integer of 0 or 1, A is one of several specified groups, such as



10 B is one of several specified groups, such as



or mixtures thereof, and n is an integer representing the number of repeating monomer units.

35

40

45

35

Aug. 29, 1996, entitled "Improved Curable Compositions," with the named inventors Timothy J. Fuller, Ram S. Narang, Thomas W. Smith, David J. Luca, and Ralph A. Mosher, and European Patent Publication 0,827,027, the disclosures of each of which are totally incorporated herein by reference, disclose an improved composition comprising a photopatternable polymer containing at least some monomer repeat units with photosensitivity-imparting substituents, said photopatternable polymer being of the general formula



65

wherein x is an integer of 0 or 1, A is one of several specified groups, such as



B is one of several specified groups, such as



or mixtures thereof, and n is an integer representing the number of repeating monomer units. Also disclosed is a process for preparing a thermal ink jet printhead with the aforementioned polymer and a thermal ink jet printhead containing therein a layer of a crosslinked or chain extended 40 polymer of the above formula.

Copending application U.S. Ser. No. 08/705,365, filed 45 Aug. 29, 1996, entitled "Hydroxyalkylated High Performance Curable Polymers," with the named inventors Ram S. Narang and Timothy J.

Fuller, and European Patent Publication 0,827,028, the disclosures of each of which are totally incorporated herein by reference, disclose a composition which comprises (a) a polymer containing at least some monomer repeat units with photosensitivity-imparting substituents which enable crosslinking or chain extension of the polymer upon exposure to actinic radiation, said polymer being of the formula



or



15 wherein x is an integer of 0 or 1, A is one of several specified groups, such as



B is one of several specified groups, such as



35

30

or mixtures thereof, and n is an integer representing the number of repeating monomer units, wherein said photosensitivity-imparting substituents are hydroxyalkyl groups; (b) at least one member selected from the group consisting of photoinitiators and sensitizers; and (c) an optional solvent. Also disclosed are processes for preparing the above polymers and methods of preparing thermal ink jet printheads containing the above polymers.

50 Copending application U.S. Ser. No. 08/705,488, filed 55 Aug. 29, 1996, entitled "Improved High Performance Polymer Compositions," with the named inventors Thomas W. Smith, Timothy J. Fuller, Ram S. Narang, and David J. Luca, and European Patent Publication 0,827,029, the disclosures of each of which are totally incorporated herein by reference, disclose a composition comprising a polymer with a weight average molecular weight of from about 1,000 60 to about 65,000, said polymer containing at least some monomer repeat units with a first, photosensitivity-imparting substituent which enables crosslinking or chain extension of the polymer upon exposure to actinic radiation,

13

said polymer also containing a second, thermal sensitivity-imparting substituent which enables further polymerization of the polymer upon exposure to temperatures of about 140° C. and higher, wherein the first substituent is not the same as the second substituent, said polymer being selected from the group consisting of polysulfones, polyphenylenes, polyether sulfones, polyimides, polyamide imides, polyarylene ethers, polyphenylene sulfides, polyarylene ether ketones, phenoxy resins, polycarbonates, polyether imides, polyquinoxalines, polyquinolines, polybenzimidazoles, polybenzoxazoles, polybenzothiazoles, polyoxadiazoles, copolymers thereof, and mixtures thereof.

Copending application U.S. Ser. No. 08/697,761, filed Aug. 29, 1996, entitled "Process for Direct Substitution of High Performance Polymers with Unsaturated Ester Groups," with the named inventors Timothy J. Fuller, Ram S. Narang, Thomas W. Smith, David J. Luca, and Raymond K. Crandall, and European Patent Publication 0,827,030, the disclosures of each of which are totally incorporated herein by reference, disclose a process which comprises reacting a polymer of the general formula



wherein x is an integer of 0 or 1, A is one of several specified groups, such as



B is one of several specified groups, such as



14



or mixtures thereof, and n is an integer representing the number of repeating monomer units, with (i) a formaldehyde source, and (ii) an unsaturated acid in the presence of an acid catalyst, thereby forming a curable polymer with unsaturated ester groups. Also disclosed is a process for preparing an ink jet printhead with the above polymer.

Copending application U.S. Ser. No. 08/705,376, filed Aug. 29, 1996, entitled "Blends Containing Curable Polymers," with the named inventors Ram S. Narang and Timothy J. Fuller, and European Patent Publication 0,827,031, the disclosures of each of which are totally incorporated herein by reference, disclose a composition which comprises a mixture of (A) a first component comprising a polymer, at least some of the monomer repeat units of which have at least one photosensitivity-imparting group thereon, said polymer having a first degree of photosensitivity-imparting group substitution measured in milliequivalents of photosensitivity-imparting group per gram and being of the general formula



wherein x is an integer of 0 or 1, A is one of several specified groups, such as



B is one of several specified groups, such as



15

-continued



or mixtures thereof, and n is an integer representing the number of repeating monomer units, and (B) a second component which comprises either (1) a polymer having a second degree of photosensitivity-imparting group substitution measured in milliequivalents of photosensitivity-imparting group per gram lower than the first degree of photosensitivity-imparting group substitution, wherein said second degree of photosensitivity-imparting group substitution may be zero, wherein the mixture of the first component and the second component has a third degree of photosensitivity-imparting group substitution measured in milliequivalents of photosensitivity-imparting group per gram which is lower than the first degree of photosensitivity-imparting group substitution and higher than the second degree of photosensitivity-imparting group substitution, or (2) a reactive diluent having at least one photosensitivity-imparting group per molecule and having a fourth degree of photosensitivity-imparting group substitution measured in milliequivalents of photosensitivity-imparting group per gram, wherein the mixture of the first component and the second component has a fifth degree of photosensitivity-imparting group substitution measured in milliequivalents of photosensitivity-imparting group per gram which is higher than the first degree of photosensitivity-imparting group substitution and lower than the fourth degree of photosensitivity-imparting group substitution; wherein the weight average molecular weight of the mixture is from about 10,000 to about 50,000; and wherein the third or fifth degree of photosensitivity-imparting group substitution is from about 0.25 to about 2 milliequivalents of photosensitivity-imparting groups per gram of mixture. Also disclosed is a process for preparing a thermal ink jet printhead with the aforementioned composition.

Copending application U.S. Ser. No. 08/705,372, filed Aug. 29, 1996, entitled "High Performance Curable Polymers and Processes for the Preparation Thereof," with the named inventors Ram S. Narang and Timothy J. Fuller, and European Patent Publication 0,827,033, the disclosures of each of which are totally incorporated herein by reference, disclose a composition which comprises a polymer containing at least some monomer repeat units with photosensitivity-imparting substituents which enable crosslinking or chain extension of the polymer upon exposure to actinic radiation, said polymer being of the formula

16



wherein x is an integer of 0 or 1, A is one of several specified groups, such as



B is one of several specified groups, such as



or mixtures thereof, and n is an integer representing the number of repeating monomer units, wherein said photosensitivity-imparting substituents are allyl ether groups, epoxy groups, or mixtures thereof. Also disclosed are a process for preparing a thermal ink jet printhead containing the aforementioned polymers and processes for preparing the aforementioned polymers.

Copending application U.S. Ser. No. 08/705,490, filed Aug. 29, 1996, entitled "Halomethylated High Performance Curable Polymers," with the named inventors Ram S. Narang and Timothy J. Fuller, the disclosure of which is totally incorporated herein by reference, discloses a process which comprises the steps of (a) providing a polymer containing at least some monomer repeat units with halomethyl group substituents which enable crosslinking or chain extension of the polymer upon exposure to a radiation

17

source which is electron beam radiation, x-ray radiation, or deep ultraviolet radiation, said polymer being of the formula



wherein x is an integer of 0 or 1, A is one of several specified groups, such as



B is one of several specified groups, such as



or mixtures thereof, and n is an integer representing the number of repeating monomer units, and (b) causing the polymer to become crosslinked or chain extended through the photosensitivity-imparting groups. Also disclosed is a process for preparing a thermal ink jet printhead by the aforementioned curing process.

Copending application U.S. Ser. No. 08/697,760, filed Aug. 29, 1996, entitled "Aqueous Developable High Performance Curable Polymers," with the named inventors Ram S. Narang and Timothy J. Fuller, and European Patent Publication 0,827,032, the disclosures of each of which are totally incorporated herein by reference, disclose a composition which comprises a polymer containing at least some monomer repeat units with water-solubility-imparting sub-

18

stituents and at least some monomer repeat units with photosensitivity-imparting substituents which enable crosslinking or chain extension of the polymer upon exposure to actinic radiation, said polymer being of the formula



25 wherein x is an integer of 0 or 1, A is one of several specified groups, such as



B is one of several specified groups, such as



55 or mixtures thereof, and n is an integer representing the number of repeating monomer units. In one embodiment, a single functional group imparts both photosensitivity and water solubility to the polymer. In another embodiment, a first functional group imparts photosensitivity to the polymer and a second functional group imparts water solubility to the polymer. Also disclosed is a process for preparing a thermal ink jet printhead with the aforementioned polymers.

Copending application U.S. Ser. No. 09/105,501, entitled "Bonding Process," with the named inventors Lisa A. DeLouise and David J. Luca, the disclosure of which is totally incorporated herein by reference, discloses a process

for bonding a first article to a second article which comprises (a) providing a first article comprising a polymer having photosensitivity-imparting substituents; (b) providing a second article comprising metal, plasma nitride, silicon, or glass; (c) applying to at least one of the first article and the second article an adhesion promoter selected from silanes, titanates, or zirconates having (i) alkoxy, aryloxy, or arylalkyloxy functional groups and (ii) functional groups including at least one photosensitive aliphatic  $>C=C<$  linkage; (d) placing the first article in contact with the second article; and (e) exposing the first article, second article, and adhesion promoter to radiation, thereby bonding the first article to the second article with the adhesion promoter. In one embodiment of the present invention, the adhesion promoter is employed in microelectrical mechanical systems such as thermal ink jet printheads.

While known compositions and processes are suitable for their intended purposes, a need remains for improved ink jet printheads. In addition, a need remains for ink jet printheads having channel plates, ink inlet plates, and/or adhesive layers between the channel plates and the insulative layers on the heater plates which are chemically inert with respect to the materials that might be employed in ink jet ink compositions. Further, a need remains for ink jet printheads with channel plates, ink inlet plates, and/or adhesive layers between the channel plates and the insulative layers on the heater plates which exhibit low shrinkage during post-cure steps in the device fabrication process. Additionally, a need remains for ink jet printheads having channel plates and/or ink inlet plates of photopatternable polymeric materials which can be patterned with relatively low photo-exposure energies. There is also a need for ink jet printheads having channel plates, ink inlet plates, and/or adhesive layers between the channel plates and the insulative layers on the heater plates which exhibit good solvent resistance. In addition, there is a need for ink jet printheads having channel plates, ink inlet plates, and/or adhesive layers between the channel plates and the insulative layers on the heater plates which exhibit reduced edge bead, no apparent lips and dips, and very low surface irregularities. Further, there is a need for ink jet printheads having channel plates, ink inlet plates, and/or adhesive layers between the channel plates and the insulative layers on the heater plates which exhibit reduced water sorption. Additionally, there is a need for ink jet printheads which have substantially no interfaces between the ink channel plates, ink inlet plates, and insulative layers on the heater plates. A need also remains for ink jet printheads which, because they have substantially no interfaces between the ink channel plates, ink inlet plates, and insulative layers on the heater plates, are resistant to attack by ink compositions, which tend to attack such interfaces. In addition, a need remains for ink jet printheads which are resistant to attack from alkaline inks.

#### SUMMARY OF THE INVENTION

It is an object of the present invention to provide ink jet printheads with the above noted advantages.

It is another object of the present invention to provide ink jet printheads having channel plates, ink inlet plates, and/or adhesive layers between the channel plates and the insulative layers on the heater plates which are chemically inert with respect to the materials that might be employed in ink jet ink compositions.

It is yet another object of the present invention to provide ink jet printheads with channel plates, ink inlet plates, and/or adhesive layers between the channel plates and the insulative layers on the heater plates which exhibit low shrinkage during post-cure steps in the device fabrication process.

It is still another object of the present invention to provide ink jet printheads having channel plates and/or ink inlet plates of photopatternable polymeric materials which can be patterned with relatively low photo-exposure energies.

Another object of the present invention is to provide ink jet printheads having channel plates, ink inlet plates, and/or adhesive layers between the channel plates and the insulative layers on the heater plates which exhibit good solvent resistance.

Yet another object of the present invention is to provide ink jet printheads having channel plates, ink inlet plates, and/or adhesive layers between the channel plates and the insulative layers on the heater plates which exhibit reduced edge bead, no apparent lips and dips, and very low surface irregularities.

Still another object of the present invention is to provide ink jet printheads having channel plates, ink inlet plates, and/or adhesive layers between the channel plates and the insulative layers on the heater plates which exhibit reduced water sorption.

It is another object of the present invention to provide ink jet printheads which have substantially no interfaces between the ink channel plates, ink inlet plates, and insulative layers on the heater plates.

It is yet another object of the present invention to provide ink jet printheads which, because they have substantially no interfaces between the ink channel plates, ink inlet plates, and insulative layers on the heater plates, are resistant to attack by ink compositions, which tend to attack such interfaces.

It is still another object of the present invention to provide ink jet printheads which are resistant to attack from alkaline inks.

These and other objects of the present invention (or specific embodiments thereof) can be achieved by providing an ink jet printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the printhead with the grooves in the upper substrate being aligned with the heating elements in the lower substrate to form droplet emitting nozzles, said upper substrate comprising a material formed by crosslinking or chain extending a polymer of the formula



21

-continued



wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of the monomer repeat units of the polymer, A is 25



or mixtures thereof, B is



22

II



55 wherein v is an integer of from 1 to about 20, and preferably from 1 to about 10.



65 wherein z is an integer of from 2 to about 20, and preferably from 2 to about 10.



wherein  $u$  is an integer of from 1 to about 20, and preferably from 1 to about 10,



wherein  $w$  is an integer of from 1 to about 20, and preferably from 1 to about 10,



or mixtures thereof, and  $n$  is an integer representing the number of repeating monomer units. In one specific embodiment, the insulative layer of the lower substrate comprises a material formed by crosslinking or chain

extending a polymer of formula I or II. In another specific embodiment, the upper substrate is bonded to the insulative layer of the lower substrate with an adhesive which comprises a material formed by crosslinking or chain extending 5 a polymer of formula I or II.

#### BRIEF DESCRIPTION OF THE DRAWINGS

FIG. 1 is an enlarged schematic isometric view of an example of a printhead mounted on a daughter board showing 10 the droplet emitting nozzles.

FIG. 2 is an enlarged cross-sectional view of FIG. 1 as viewed along the line 2—2 thereof and showing the electrode passivation and ink flow path between the manifold and the ink channels. 15

FIG. 3 is an enlarged cross-sectional view of an alternate embodiment of the printhead in FIG. 1 as viewed along the line 2—2 thereof.

#### DETAILED DESCRIPTION OF THE 20 INVENTION

The present invention is directed to an ink jet printhead which comprises (i) an upper substrate with a set of parallel grooves for subsequent use as ink channels and a recess for 25 subsequent use as a manifold, the grooves being open at one end for serving as droplet emitting nozzles, and (ii) a lower substrate in which one surface thereof has an array of heating elements and addressing electrodes formed thereon, 30 said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the 35 printhead with the grooves in the upper substrate being aligned with the heating elements in the lower substrate to form droplet emitting nozzles, said upper substrate comprising a material formed by crosslinking or chain extending a polymer of formula I or II. An example of a suitable 40 configuration, suitable in this instance for thermal ink jet printing, is illustrated schematically in FIG. 1, which depicts an enlarged, schematic isometric view of the front face 29 of a printhead 10 showing the array of droplet emitting nozzles 27. Referring also to FIG. 2, discussed later, the lower 45 electrically insulating substrate or heating element plate 28 has the heating elements 34 and addressing electrodes 33 patterned on surface 30 thereof, while the upper substrate or channel plate 31 has parallel grooves 20 which extend in one direction and penetrate through the upper substrate front 50 face edge 29. The other end of grooves 20 terminate at slanted wall 21, the floor 41 of the internal recess 24 which is used as the ink supply manifold for the capillary filled ink channels 20, has an opening 25 therethrough for use as an ink fill hole. The surface of the channel plate with the 55 grooves are aligned and bonded to the heater plate 28, so that a respective one of the plurality of heating elements 34 is positioned in each channel, formed by the grooves and the lower substrate or heater plate. Ink enters the manifold formed by the recess 24 and the lower substrate 28 through 60 the fill hole 25 and by capillary action, fills the channels 20 by flowing through an elongated recess 38 formed in the thick film insulative layer 18. The ink at each nozzle forms a meniscus, the surface tension of which prevents the ink from weeping therefrom. The addressing electrodes 33 on the lower substrate or channel plate 28 terminate at terminals 65 32. The upper substrate or channel plate 31 is smaller than that of the lower substrate in order that the electrode

terminals 32 are exposed and available for wire bonding to the electrodes on the daughter board 19, on which the printhead 10 is permanently mounted. Layer 18, discussed later, is a thick film passivation layer sandwiched between the upper and lower substrates. This layer is etched to expose the heating elements, thus placing them in a pit, and is etched to form the elongated recess to enable ink flow between the manifold 24 and the ink channels 20. In addition, the thick film insulative layer is etched to expose the electrode terminals.

A cross sectional view of FIG. 1 is taken along view line 2—2 through one channel and shown as FIG. 2 to show how the ink flows from the manifold 24 and around the end 21 of the groove 20 as depicted by arrow 23. As is disclosed in U.S. Pat. Nos. 4,638,337, 4,601,777, and U.S. Pat. No. Re. 32,572, the disclosures of each of which are totally incorporated herein by reference, a plurality of sets of bubble generating heating elements 34 and their addressing electrodes 33 can be patterned on the polished surface of a single side polished (100) silicon wafer. Prior to patterning, the multiple sets of printhead electrodes 33, the resistive material that serves as the heating elements 34, and the common return 35, the polished surface of the wafer is coated with an underglaze layer 39 such as silicon dioxide, having a typical thickness of from about 5,000 Angstroms to about 2 microns, although the thickness can be outside this range. The resistive material can be a doped polycrystalline silicon, which can be deposited by chemical vapor deposition (CVD) or any other well known resistive material such as zirconium boride (ZrB<sub>2</sub>). The common return and the addressing electrodes are typically aluminum leads deposited on the underglaze and over the edges of the heating elements. The common return ends or terminals 37 and addressing electrode terminals 32 are positioned at predetermined locations to allow clearance for wire bonding to the electrodes (not shown) of the daughter board 19, after the channel plate 31 is attached to make a printhead. The common return 35 and the addressing electrodes 33 are deposited to a thickness typically of from about 0.5 to about 3 microns, although the thickness can be outside this range, with the preferred thickness being 1.5 microns.

If polysilicon heating elements are used, they may be subsequently oxidized in steam or oxygen at a relatively high temperature, typically about 1,100° C. although the temperature can be above or below this value, for a period of time typically of from about 50 to about 80 minutes, although the time period can be outside this range, prior to the deposition of the aluminum leads, in order to convert a small portion of the polysilicon to SiO<sub>2</sub>. In such cases, the heating elements are thermally oxidized to achieve an overglaze (not shown) of SiO<sub>2</sub> with a thickness typically of from about 500 Angstroms to about 1 micron, although the thickness can be outside this range, which has good integrity with substantially no pinholes.

In one embodiment, polysilicon heating elements are used and an optional silicon dioxide thermal oxide layer 17 is grown from the polysilicon in high temperature steam. The thermal oxide layer is typically grown to a thickness of from about 0.5 to about 1 micron, although the thickness can be outside this range, to protect and insulate the heating elements from the conductive ink. The thermal oxide is removed at the edges of the polysilicon heating elements for attachment of the addressing electrodes and common return, which are then patterned and deposited. If a resistive material such as zirconium boride is used for the heating elements, then other suitable well known insulative materials can be used for the protective layer thereover. Before

electrode passivation, a tantalum (Ta) layer (not shown) can be optionally deposited, typically to a thickness of about 1 micron, although the thickness can be above or below this value, on the heating element protective layer 17 for added protection thereof against the cavitation forces generated by the collapsing ink vapor bubbles during printhead operation. The tantalum layer is etched off all but the protective layer 17 directly over the heating elements using, for example, CF<sub>4</sub>/O<sub>2</sub> plasma etching. For polysilicon heating elements, the aluminum common return and addressing electrodes typically are deposited on the underglaze layer and over the opposing edges of the polysilicon heating elements which have been cleared of oxide for the attachment of the common return and electrodes.

For electrode passivation, a film 16 is deposited over the entire wafer surface, including the plurality of sets of heating elements and addressing electrodes. The passivation film 16 provides an ion barrier which will protect the exposed electrodes from the ink. Examples of suitable ion barrier materials for passivation film 16 include polyimide, plasma nitride, phosphorous doped silicon dioxide, materials disclosed hereinafter as being suitable for insulative layer 18, and the like, as well as any combinations thereof. An effective ion barrier layer is generally achieved when its thickness is from about 1000 Angstroms to about 10 microns, although the thickness can be outside this range. In 300 dpi printheads, passivation layer 16 preferably has a thickness of about 3 microns, although the thickness can be above or below this value. In 600 dpi printheads, the thickness of passivation layer 16 preferably is such that the combined thickness of layer 16 and layer 18 is about 25 microns, although the thickness can be above or below this value. The passivation film or layer 16 is etched off of the terminal ends of the common return and addressing electrodes for wire bonding later with the daughter board electrodes. This etching of the silicon dioxide film can be by either the wet or dry etching method. Alternatively, the electrode passivation can be by plasma deposited silicon nitride (Si<sub>3</sub>N<sub>4</sub>).

Next, a thick film type insulative layer 18 is formed on the passivation layer 16, typically having a thickness of from about 10 to about 100 microns and preferably in the range of from about 25 to about 50 microns, although the thickness can be outside these ranges. Layer 18 can be made of any suitable or desired photopatternable material, such as Riston®, Vacrel®, Probimer®, polyimides, including (but not limited to) those disclosed in, for example, U.S. Pat. No. 5,773,553, the disclosure of which is totally incorporated herein by reference, photoactive polyarylene ether-type materials, or the like. Preferably, layer 18 is formulated of one of the materials discussed herein as suitable for channel plate 31, and even more preferably, is of the same material as channel plate 31; when channel plate 31 and layer 18 are of the same material, the interface between channel plate 31 and layer 18 can be eliminated. Even more preferably, in 300 dpi printheads, layer 18 preferably has a thickness of about 40 microns, and in 600 dpi printheads, layer 18 preferably has a thickness of from about 20 to about 22 microns, although other thicknesses can be employed. The insulative layer 18 is photolithographically processed to enable etching and removal of those portions of the layer 18 over each heating element (forming recesses 26), the elongated recess 38 for providing ink passage from the manifold 24 to the ink channels 20, and over each electrode terminal 32, 37. The elongated recess 38 is formed by the removal of this portion of the thick film layer 18. Thus, the passivation layer 16 alone protects the electrodes 33 from exposure to the ink in

this elongated recess **38**. Optionally, if desired, insulative layer **18** can be applied as a series of thin layers of either similar or different composition. Typically, a thin layer is deposited, photoexposed, partially cured, followed by deposition of the next thin layer, photoexposure, partial curing, and the like. In one embodiment of the present invention, a first thin layer is applied to contact layer **16**, said first thin layer containing a mixture of a photopatternable material and an epoxy polymer, followed by photoexposure, partial curing, and subsequent application of one or more successive thin layers containing a photopatternable material.

In one embodiment, a heater wafer with a phosphosilicate glass layer is spin coated with a solution of Z6020 adhesion promoter (0.01 weight percent in 95 parts methanol and 5 parts water, Dow Corning) at 3000 revolutions per minute for 10 seconds and dried at 100° C. for between 2 and 10 minutes. The wafer is then allowed to cool at 25° C. for 5 minutes before spin coating the photoresist containing the photopatternable polymer onto the wafer at between 1,000 and 3,000 revolutions per minute for between 30 and 60 seconds. The photoresist solution is made by dissolving polyarylene ether ketone with 0.75 acryloyl groups and 0.75 chloromethyl groups per repeat unit and a weight average molecular weight ( $M_w$ ) of from about 15,000 to about 20,000 in N-methylpyrrolidinone at 40 weight percent solids with Michler's ketone (1.2 parts ketone per every 10 parts of 40 weight percent solids polymer solution). The film is heated (soft baked) in an oven for between 10 and 15 minutes at 80° C. After cooling to 25° C. over 5 minutes, the film is covered with a mask and exposed to 365 nanometer ultraviolet light, amounting to between 150 and 1500 millijoules per cm<sup>2</sup>. The exposed wafer is then heated at 70 to 80° C. for 2 minutes post exposure bake, followed by cooling to 25° C. over 5 minutes. The film is developed with 60:40 chloroform/cyclohexanone developer, washed with 90:10 hexanes/cyclohexanone, and then dried at 70 to 80° C. for 2 minutes. A second developer/wash cycle is carried out if necessary to obtain a wafer with clean features. The processed wafer is transferred to an oven at 25° C., and the oven temperature is raised from 25 to 90° C. at 2° C. per minute. The temperature is maintained at 90° C. for 2 hours, and then increased to 260° C. at 2° C. per minute. The oven temperature is maintained at 260° C. for 2 hours and then the oven is turned off and the temperature is allowed to cool gradually to 25° C. When thermal cure of the photoresist films is carried out under an inert atmosphere, such as nitrogen or one of the noble gases, such as argon, neon, krypton, xenon, or the like, there is markedly reduced oxidation of the developed film and improved thermal and hydrolytic stability of the resultant devices. Moreover, adhesion of developed photoresist film is improved to the underlying substrate. If a second layer is spin coated over the first layer, the heat cure of the first developed layer can be stopped at about 80° C. before the second layer is spin coated onto the first layer. A second thicker layer is deposited by repeating the above procedure a second time. This process is intended to be a guide in that procedures can be outside the specified conditions depending on film thickness and photoresist molecular weight. Films at 30 microns have been developed with clean features at 600 dots per inch. In a preferred embodiment of the present invention, the heat cure of layer **18** is stopped at about 80° C. and channel plate **31** is bonded to layer **18**, followed by thermal cure of both layer **18** and channel plate **31**, thereby resulting in formation of an interface-free bond between layer **18** and channel plate **31**.

FIG. 3 is a similar view to that of FIG. 2 with a shallow anisotropically etched groove **40** in the heater plate, which

is silicon, prior to formation of the underglaze **39** and patterning of the heating elements **34**, electrodes **33** and common return **35**. This recess **40** permits the use of only the thick film insulative layer **18** and eliminates the need for the usual electrode passivating layer **16**. Since the thick film layer **18** is impervious to water and relatively thick (typically from about 20 to about 40 microns, although the thickness can be outside of this range), contamination introduced into the circuitry will be much less than with only the relatively thin passivation layer **16** well known in the art. The heater plate is a fairly hostile environment for integrated circuits. Commercial ink generally entails a low attention to purity. As a result, the active part of the heater plate will be at elevated temperature adjacent to a contaminated aqueous ink solution which undoubtedly abounds with mobile ions. In addition, it is generally desirable to run the heater plate at a voltage of from about 30 to about 50 volts, so that there will be a substantial field present. Thus, the thick film insulative layer **18** provides improved protection for the active devices and provides improved protection, resulting in longer operating lifetime for the heater plate.

When a plurality of lower substrates **28** are produced from a single silicon wafer, at a convenient point after the underglaze is deposited, at least two alignment markings **25** (not shown) preferably are photolithographically produced at predetermined locations on the lower substrates **28** which make up the silicon wafer. These alignment markings are used for alignment of the plurality of upper substrates **31** containing the ink channels. The surface of the single sided wafer containing the plurality of sets of heating elements is bonded to the surface of the wafer containing the plurality of ink channel containing upper substrates subsequent to alignment.

In one embodiment of the present invention, by methods similar to those disclosed in U.S. Pat. Nos. 4,601,777 and 4,638,337, the disclosures of each of which are totally incorporated herein by reference, the channel plate is formed from a two side polished, (100) silicon wafer to produce a plurality of upper substrates **31** for the printhead. After the wafer is chemically cleaned, a layer of the polymer of Formula I or II as detailed further hereinbelow is deposited on both sides. Using photolithographic techniques as described hereinabove with respect to layer **18**, a via for fill hole **25** for each of the plurality of channel plates **31** and at least two vias for alignment openings (not shown) at predetermined locations are formed on one wafer side. The photopatternable polymer is exposed and removed from the patterned vias representing the fill holes and alignment openings. A potassium hydroxide (KOH) anisotropic etch **50** can be used to etch the fill holes and alignment openings. In this case, the (111) planes of the (100) wafer typically make an angle of about 54.7 degrees with the surface of the wafer. The fill holes are small square surface patterns, typically of about 20 mils (500 microns) per side, although the dimensions can be above or below this value, and the alignment openings typically are from about 60 to about 80 mils (1.5 to 3 millimeters) square, although the dimensions can be outside this range. Thus, the alignment openings are etched entirely through the 20 mil (0.5 millimeter) thick wafer, while the fill holes are etched to a terminating apex at about halfway through to three-quarters through the wafer. The relatively small square fill hole is invariant to further size increase with continued etching so that the etching of the alignment openings and fill holes are not significantly time constrained. Next, the opposite side of the wafer is photolithographically patterned, using the previously etched alignment holes as a reference to form the relatively large

rectangular recesses **24** and sets of elongated, parallel channel recesses that will eventually become the ink manifolds and channels of the printheads. The free standing channel plate **31** can then be bonded to the heater plate **28**. In a preferred embodiment of the present invention, the heat cure of both layer **18** and channel plate **31** is stopped at about 80° C. and channel plate **31** is bonded to layer **18**, followed by thermal cure of both layer **18** and channel plate **31**, thereby resulting in formation of an interface-free bond between layer **18** and channel plate **31**. In this embodiment, the portion of channel plate **31** in which the ink channels are formed, i.e., that portion of channel plate **31** below dotted line **65** in FIGS. 2 and 3, is formed of the polymer of Formula I or II, and the portion of channel plate **31** in which the ink fill hole **25** is formed, i.e., that portion of channel plate **31** above dotted line **65** in FIGS. 2 and 3, is formed of silicon.

In another embodiment of the present invention, the channel plate is formed by applying to one surface of the silicon wafer a layer of the polymer of Formula I or II as detailed further hereinbelow and a layer of silicon nitride to the other surface of the silicon wafer. Using photolithographic techniques, a via for fill hole **25** for each of the plurality of channel plates **31** and at least two vias for alignment openings (not shown) at predetermined locations are etched in the silicon nitride on one wafer side. The silicon nitride is etched from the patterned vias representing the fill holes and alignment openings. A potassium hydroxide (KOH) anisotropic etch can be used to etch the fill holes and alignment openings. In this case, the (111) planes of the (100) wafer typically make an angle of about 54.7 degrees with the surface of the wafer. The fill holes are small square surface patterns, typically of about 20 mils (500 microns) per side, although the dimensions can be above or below this value, and the alignment openings typically are from about 60 to about 80 mils (1.5 to 3 millimeters) square, although the dimensions can be outside this range. Thus, the alignment openings are etched entirely through the 20 mil (0.5 millimeter) thick wafer, while the fill holes are etched to a terminating apex at about halfway through to three-quarters through the wafer. The relatively small square fill hole is invariant to further size increase with continued etching so that the etching of the alignment openings and fill holes are not significantly time constrained. Next, the opposite side of the wafer is photolithographically patterned, using the previously etched alignment holes as a reference to form the relatively large rectangular recesses **24** and sets of elongated, parallel channel recesses that will eventually become the ink manifolds and channels of the printheads. The free standing channel plate **31** can then be bonded to the heater plate **28**. In a preferred embodiment of the present invention, the heat cure of both layer **18** and channel plate **31** is stopped at about 80° C. and channel plate **31** is bonded to layer **18**, followed by thermal cure of both layer **18** and channel plate **31**, thereby resulting in formation of an interface-free bond between layer **18** and channel plate **31**. In this embodiment, the portion of channel plate **31** in which the ink channels are formed, i.e., that portion of channel plate **31** below dotted line **65** in FIGS. 2 and 3, is formed of the polymer of Formula I or II, and the portion of channel plate **31** in which the ink fill hole **25** is formed, i.e., that portion of channel plate **31** above dotted line **65** in FIGS. 2 and 3, is formed of silicon.

In yet another embodiment of the present invention, the channel plate **31** is formed by coating a glass plate with a layer of an adhesion promoter. Examples of suitable adhesion promoters include dialkoxy silanes and trialkoxy

silanes, such as N-( $\beta$ -aminoethyl)- $\gamma$ -aminopropyltrimethoxysilane (Z-6020, available from Dow Corning, Midland, Mich.), of the formula  $(CH_3O)_3SiCH_2CH_2CH_2NHCH_2CH_2NH_2$ , 0.01 weight percent in 95 parts methanol and 5 parts water, and the like. Coating of the glass plate with the adhesion promoter typically takes place by spin coating at about 3,000 rpm, followed by heating to about 100° C. and maintaining the plate at this temperature for a period of about 10 minutes to ensure that the molecules of the adhesion promoter have crosslinked to form a water resistant network, and then allowing the coated plate to cool to room temperature. Thereafter, a thick film (typically from about 20 to about 50 microns, and preferably about 40 microns, although the thickness can be outside of this range) of a polymer of Formula I or II is applied to the top of the film of adhesion promoter by any desired or suitable method, such as spin coating, doctor blading, or the like. The coated plate is then transferred to a heating device, such as a hot plate, typically at a temperature of about 75° C. for a polyarylene ether ketone polymer having a weight average molecular weight of about 16,000, about 0.75 acryloyl groups per repeat monomer unit, and about 1.5 chloromethyl groups per repeat monomer unit, until the film of photopatternable polymer is dry to the touch. The dried photopatternable film is then exposed to radiation at a wavelength to which it is sensitive to enable crosslinking or chain extension (365 nanometers, for example, for a polyarylene ether ketone polymer having a weight average molecular weight of about 16,000, about 0.75 acryloyl groups per repeat monomer unit, and about 1.5 chloromethyl groups per repeat monomer unit) through an appropriate mask, thereby patterning the ink channels **20** and the ink fill holes **25**. Following exposure, the film is heated to a temperature of about 100° C. and maintained at that temperature for one hour, to advance the polymerization of exposed areas of the polymer to the stage where the exposed areas will not dissolve and the unexposed areas will dissolve upon development, followed by raising the temperature at a rate of 2° C. per minute to 260° C. and then maintaining the temperature at 260° C. for 2 hours to ensure almost complete crosslinking of the film. At this point, the film can be removed from the glass plate by dipping it for a few minutes in a solvent appropriate for the adhesion promoter, such as a mixture of water and imidazole of pH about 9 or higher, and separating the film from the glass plate. The free standing channel plate **31** can then be bonded to the heater plate **28**. Alternatively, the channel plate **31** can be bonded to the heater plate **28** while still attached to the glass plate, followed by removal of the glass plate by dipping the assembly in the aforementioned solvent and separating the glass plate from the channel plate. In a preferred embodiment of the present invention, the heat cure of both layer **18** and channel plate **31** is stopped at about 80° C. and channel plate **31** is bonded to layer **18**, followed by thermal cure of both layer **18** and channel plate **31**, thereby resulting in formation of an interface-free bond between layer **18** and channel plate **31**. In this embodiment, both the portion of channel plate **31** in which the ink channels are formed, i.e., that portion of channel plate **31** below dotted line **65** in FIGS. 2 and 3, and the portion of channel plate **31** in which the ink fill hole **25** is formed, i.e., that portion of channel plate **31** above dotted line **65** in FIGS. 2 and 3, are formed of the polymer of Formula I or II.

In still another embodiment, the channel plate **31** is formed in two stages. A glass plate is coated with a layer of an adhesion promoter and heated as described above. Thereafter, a somewhat thinner film (typically from about 10

to about 20 microns, and preferably about 20 microns, although the thickness can be outside of this range) of a polymer of Formula I or II is applied to the top of the film of adhesion promoter by any desired or suitable method, such as spin coating, doctor blading, or the like. The coated plate is then transferred to a heating device, such as a hot plate, typically at a temperature of about 100° C. for a period typically of from about 0.1 to about 1 hour. The dried photopatternable film is then exposed to radiation at a wavelength at which it is sensitive to crosslinking or chain extension (365 nanometers, for example, for a polyarylene ether ketone polymer having a weight average molecular weight of about 16,000, about 0.75 acryloyl groups per repeat monomer unit, and about 1.5 chloromethyl groups per repeat monomer unit) through an appropriate mask, thereby patterning the ink channels 20. Thereafter, a second layer (typically from about 20 to about 30 microns, and preferably about 30 microns, although the thickness can be outside of this range) of a polymer of Formula I or II is applied to the top of the film of adhesion promoter by any desired or suitable method, such as spin coating, doctor blading, or the like. The coated plate is then transferred to a heating device, such as a hot plate, typically at a temperature of about 75° C. until the second film of photopatternable polymer is dry to the touch. The dried photopatternable film is then exposed to radiation at a wavelength at which it is sensitive to crosslinking or chain extension (365 nanometers, for example, for a polyarylene ether ketone polymer having a weight average molecular weight of about 16,000, about 0.75 acryloyl groups per repeat monomer unit, and about 1.5 chloromethyl groups per repeat monomer unit) through an appropriate mask, thereby patterning the ink fill holes 25. Following exposure, the films are heated to a temperature of about 100° C. and maintained at that temperature for one hour. This initial annealing at about 100° C. enables the intermingling of the two layers, thereby eliminating any interface between them. Thereafter, the temperature is raised at a rate of 2° C. per minute to 260° C. and then maintained at 260° C. for 2 hours to ensure almost complete crosslinking of the film. At this point, the film can be removed from the glass plate by dipping it for a few minutes in a solvent appropriate for the adhesion promoter, such as a mixture of water and imidazole of pH about 9 or higher, and separating the film from the glass plate. The free standing channel plate 31 can then be bonded to the heater plate 28. Alternatively, the channel plate 31 can be bonded to the heater plate 28 while still attached to the glass plate, followed by removal of the glass plate by dipping the assembly in the aforementioned solvent and separating the glass plate from the channel plate. In a preferred embodiment of the present invention, the heat cure of both layer 18 and channel plate 31 is stopped at about 80° C. and channel plate 31 is bonded to layer 18, followed by thermal cure of both layer 18 and channel plate 31, thereby resulting in formation of an interface-free bond between layer 18 and channel plate 31. In this embodiment, both the portion of channel plate 31 in which the ink channels are formed, i.e., that portion of channel plate 31 below dotted line 65 in FIGS. 2 and 3, and the portion of channel plate 31 in which the ink fill hole 25 is formed, i.e., that portion of channel plate 31 above dotted line 65 in FIGS. 2 and 3, are formed of the polymer of Formula I or II.

The surface 22 of the wafer containing the manifold and channel recesses are portions of the original wafer surface on which an adhesive, such as a thermosetting epoxy, will be applied later for bonding it to the substrate containing the plurality of sets of heating elements. The adhesive is applied

in a manner such that it does not run or spread into the grooves or other recesses. The alignment markings can be used with, for example, a vacuum chuck mask aligner to align the channel wafer on the heating element and addressing electrode wafer. The two wafers are accurately mated and can be tacked together by partial curing of the adhesive. Alternatively, the heating element and channel wafers can be given precisely diced edges and then manually or automatically aligned in a precision jig. Alignment can also be performed with an infrared aligner-bonder, with an infrared microscope using infrared opaque markings on each wafer to be aligned, or the like. The two wafers can then be cured in an oven or laminator to bond them together permanently. The channel wafer can then be milled to produce individual upper substrates. A final dicing cut, which produces end face 29, opens one end of the elongated groove 20 producing nozzles 27. The other ends of the channel groove 20 remain closed by end 21. However, the alignment and bonding of the channel plate to the heater plate places the ends 21 of channels 20 directly over elongated recess 38 in the thick film insulative layer 18 as shown in FIG. 2 or directly above the recess 40 as shown in FIG. 3 enabling the flow of ink into the channels from the manifold as depicted by arrows 23. The plurality of individual printheads produced by the final dicing are bonded to the daughter board and the printhead electrode terminals are wire bonded to the daughter board electrodes.

In a preferred embodiment, instead of bonding the heater plate to the channel plate with an adhesive such as an epoxy, a polymer of Formula I or II is used to bond the heater plate to the channel plate. Preferably, layer 18 of the heater plate, channel plate, and adhesive are all of the same polymer, although it may be desired in some instances to vary the characteristics of the polymer for the different applications; for example, the polymer used as the adhesive may be of somewhat lower molecular weight, and may have a somewhat higher number of photosensitivity-imparting substituents per repeat monomer unit than the polymer used for layer 18 of the heater plate and for channel plate 31. In this embodiment, layer 18 of a photopatternable polyarylene ether-type polymer is applied to the heater plate in the desired thickness, followed by photopatterning to expose the heating elements. The patterned layer 18 is subjected to an initial post-exposure heating, typically at temperatures of about 120° C. for about 1 hour, but is not completely cured. Channel plate 31 is prepared of photopatternable polyarylene ether-type polymer by one of the methods described above, and is subjected to an initial post-exposure heating, typically at temperatures of about 120° C. for about 1 hour, but is not completely cured. Thereafter, a thin film, typically of from about 1 to about 2 microns, of a photopatternable polyarylene ether-type polymer is applied to either the heater plate or the channel plate, either directly or indirectly by first applying it to a substrate such as a Mylar® polyester disc and then transferring it from the disc to either the heater plate or the channel plate. The heater plate and the channel plate are then aligned, and the entire assembly is annealed under a hydrostatic pressure typically of from about 30 to about 50 pounds per square inch, preferably under an inert atmosphere such as nitrogen, at a temperature of from about 200 to about 250° C. for a period of about 2 hours. The resulting printhead is free of seams and interfaces between the heater plate and the channel plate.

The printhead illustrated in FIGS. 1 through 3 constitutes a specific embodiment of the present invention. Any other suitable printhead configuration comprising ink-bearing channels terminating in nozzles on the printhead surface can

also be employed with the materials disclosed herein to form a printhead of the present invention.

For best results with respect to well-resolved features and high aspect ratios, the photopatternable polyarylene ether-type compositions of the present invention are free of particulates prior to coating onto substrates. In one preferred embodiment, the photoresist composition containing the photopatternable polymer is subjected to filtration through a 2 micron nylon filter cloth (available from Tetko). The photoresist solution is filtered through the cloth under yellow light or in the dark as a solution containing from about 30 to about 60 percent by weight solids using compressed air (up to about 60 psi) and a pressure filtration funnel. No dilution of the photoresist solution is required, and concentrations of an inhibitor (such as, for example, MEHQ) can be as low as, for example, 500 parts per million or less by weight without affecting shelf life. No build in molecular weight of the photopatternable polymer is observed during this filtration process. While not being limited to any particular theory, it is believed that in some instances, such as those when unsaturated ester groups are present on the photopolymerizable polymer, compressed air yields results superior to those obtainable with inert atmosphere because oxygen in the compressed air acts as an effective inhibitor for the free radical polymerization of unsaturated ester groups such as acrylates and methacrylates.

The photopatternable polymer used for the channel plate (and, in some embodiments of the present invention, for insulative layer 18 of the heater plate and/or for the adhesive between the channel plate and the insulative layer of the heater plate) is of the general formula 30



wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of the monomer repeat units of the polymer, A is

35



wherein v is an integer of from 1 to about 20, and preferably from 1 to about 10,



36



wherein w is an integer of from 1 to about 20, and preferably from 1 to about 10,



40 other similar bisphenol derivatives, or mixtures thereof, and n is an integer representing the number of repeating monomer units. The value of n is such that the weight average molecular weight of the material is from about 1,000 to about 100,000, preferably from about 1,000 to about 65,000, more preferably from about 1,000 to about 40,000, and even more preferably from about 3,000 to about 25,000, although the weight average molecular weight can be outside these ranges. Preferably, n is an integer of from about 2 to about 70, more preferably from about 5 to about 70, and even more preferably from about 8 to about 50, although the value of n can be outside these ranges. The phenyl groups and the A and/or B groups may also be substituted, although the presence of two or more substituents on the B group ortho to the oxygen groups can render substitution difficult. Substituents can be present on the polymer either prior to or subsequent to the placement of photosensitivity-imparting functional groups thereon. Substituents can also be placed on the polymer during the process of placement of photosensitivity-imparting functional groups thereon.

45 Examples of suitable substituents include (but are not limited to) alkyl groups, including saturated, unsaturated, and cyclic alkyl groups, preferably with from 1 to about 6 carbon atoms, substituted alkyl groups, including saturated, unsaturated, and cyclic substituted alkyl groups, preferably with from 1 to about 6 carbon atoms, aryl groups, preferably with from 6 to about 24 carbon atoms, substituted aryl groups, preferably with from 6 to about 24 carbon atoms,

50

55

60

65

arylalkyl groups, preferably with from 7 to about 30 carbon atoms, substituted arylalkyl groups, preferably with from 7 to about 30 carbon atoms, alkoxy groups, preferably with from 1 to about 6 carbon atoms, substituted alkoxy groups, preferably with from 1 to about 6 carbon atoms, aryloxy groups, preferably with from 6 to about 24 carbon atoms, substituted aryloxy groups, preferably with from 6 to about 24 carbon atoms, arylalkyloxy groups, preferably with from 7 to about 30 carbon atoms, substituted arylalkyloxy groups, preferably with from 7 to about 30 carbon atoms, hydroxy groups, amine groups, imine groups, ammonium groups, pyridine groups, pyridinium groups, ether groups, ester groups, amide groups, carbonyl groups, thiocarbonyl groups, sulfate groups, sulfonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein two or more substituents can be joined together to form a ring, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein two or more substituents can be joined together to form a ring. Processes for the preparation of these materials are known, and disclosed in, for example, P. M. Hergenrother, *J. Macromol. Sci. Rev. Macromol. Chem.*, C19 (1), 1-34 (1980); P. M. Hergenrother, B. J. Jensen, and S. J. Havens, *Polymer*, 29, 358 (1988); B. J. Jensen and P. M. Hergenrother, "High Performance Polymers," Vol. 1, No. 1 page 31 (1989), "Effect of Molecular Weight on Poly (arylene ether ketone) Properties"; V. Percec and B. C. Auman, *Makromol. Chem.* 185, 2319 (1984); "High Molecular Weight Polymers by Nickel Coupling of Aryl Polychlorides," I. Colon, G. T. Kwiatkowski, *J. of Polymer Science, Part A: Polymer Chemistry*, 28 367 (1990); M. Ueda and T. Ito, *Polymer J.*, 23 (4), 297 (1991); "Ethynyl-Terminated Polyarylates: Synthesis and Characterization," S. J. Havens and P. M. Hergenrother, *J. of Polymer Science: Polymer Chemistry Edition*, 22, 3011 (1984); "Ethynyl-Terminated Polysulfones: Synthesis and Characterization," P. M. Hergenrother, *J. of Polymer Science: Polymer Chemistry Edition*, 20, 3131 (1982); K. E. Dukes, M. D. Forbes, A. S. Jeevarajan, A. M. Belu, J. M. DeDimone, R. W. Linton, and V. V. Sheares, *Macromolecules*, 29, 3081 (1996); G. Hougham, G. Tesoro, and J. Shaw, *Polym. Mater. Sci. Eng.*, 61, 369 (1989); V. Percec and B. C. Auman, *Makromol. Chem.* 185, 617 (1984); "Synthesis and characterization of New Fluorescent Poly(arylene ethers)," S. Matsuo, N. Yakoh, S. Chino, M. Mitani, and S. Tagami, *Journal of Polymer Science: Part A: Polymer Chemistry*, 32, 1071 (1994); "Synthesis of a Novel Naphthalene-Based Poly (arylene ether ketone) with High Solubility and Thermal Stability," Mami Ohno, Toshikazu Takata, and Takeshi Endo, *Macromolecules*, 27 3447 (1994); "Synthesis and Characterization of New Aromatic Poly(ether ketones)," F. W. Mercer, M. T. Mckenzie, G. Merlino, and M. M. Fone, *J. of Applied Polymer Science*, 56, 1397 (1995); H. C.

Zhang, T. L. Chen, Y. G. Yuan, Chinese Patent CN 85108751 (1991); "Static and laser light scattering study of novel thermoplastics. 1. Phenolphthalein poly(aryl ether ketone)," C. Wu, S. Bo, M. Siddiq, G. Yang and T. Chen, *Macromolecules*, 29 2989 (1996); "Synthesis of t-Butyl-Substituted Poly(ether ketone) by Nickel-Catalyzed Coupling Polymerization of Aromatic Dichloride", M. Ueda, Y. Seino, Y. Haneda, M. Yoneda, and J.-I. Sugiyama, *Journal of Polymer Science: Part A: Polymer Chemistry*, 32, 675 (1994); "Reaction Mechanisms: Comb-Like Polymers and Graft Copolymers from Macromers 2. Synthesis, Characterization and Homopolymerization of a Styrene Macromer of Poly(2,6-dimethyl-1,4-phenylene Oxide)," V. Percec, P. L. Rinaldi, and B. C. Auman, *Polymer Bulletin*, 10, 397 (1983); *Handbook of Polymer Synthesis Part A*, Hans R. Kricheldorf, ed., Marcel Dekker, Inc., New York-Basel-Hong Kong (1992); and "Introduction of Carboxyl Groups into Crosslinked Polystyrene," C. R. Harrison, P. Hodge, J. Kemp, and G. M. Perry, *Die Makromolekulare Chemie*, 176, 267 (1975), the disclosures of each of which are totally incorporated herein by reference. Further background on high performance polymers is disclosed in, for example, U.S. Pat. Nos. 2,822,351; 3,065,205; British Patent 1,060,546; British Patent 971,227; British Patent 1,078,234; U.S. Pat. No. 4,175,175; N. Yoda and H. Hiramoto, *J. Macromol. Sci.-Chem.*, A21(13 & 14) pp. 1641 (1984) (Toray Industries, Inc., Otsu, Japan; B. Sillion and L. Verdet, "Polyimides and other High-Temperature polymers", edited by M. J. M. Abadie and B. Sillion, Elsevier Science Publishers B.V. (Amsterdam 1991); "Polyimides with Alicyclic Diamines. 1. Hydrogen Abstraction and Photocrosslinking Reactions of Benzophenone Type Polyimides," Q. Jin, T. Yamashita, and K. Horie, *J. of Polymer Science: Part A: Polymer Chemistry*, 32, 503 (1994); Probimide™ 300, product bulletin, Ciba-Geigy Microelectronics Chemicals, "Photosensitive Polyimide System," *High Performance Polymers and Composites*, J. I. Kroschwitz (ed.), John Wiley & Sons (New York 1991); and T. E. Atwood, D. A. Barr, T. A. King, B. Newton, and B. J. Rose, *Polymer*, 29, 358 (1988), the disclosures of each of which are totally incorporated herein by reference. Further information on radiation curing is disclosed in, for example, *Radiation Curing: Science and Technology*, S. Peter Pappas, ed., Plenum Press (New York 1992), the disclosure of which is totally incorporated herein by reference. Polymers of these formulae, the preparation thereof, and the use thereof as photopatternable polymers in layer 18 of thermal ink jet printheads are disclosed in, for example, U.S. Pat. No. 5,739,254, copending application U.S. Ser. No. 08/705,375, filed Aug. 29, 1996, copending application U.S. Ser. No. 08/705,365, filed Aug. 29, 1996, copending application U.S. Ser. No. 08/705,488, filed Aug. 29, 1996, copending application U.S. Ser. No. 08/697,761, filed Aug. 29, 1996, copending application U.S. Ser. No. 08/705,479, filed Aug. 29, 1996, copending application U.S. Ser. No. 08/705,376, filed Aug. 29, 1996, copending application U.S. Ser. No. 08/705,372, filed Aug. 29, 1996, copending application U.S. Ser. No. 08/705,490, filed Aug. 29, 1996, copending application U.S. Ser. No. 08/697,760, filed Aug. 29, 1996, copending application U.S. Ser. No. 08/920,240, filed Aug. 28, 1997, European Patent Publication 0,826,700, European Patent Publication 0,827,027, European Patent Publication 0,827,028, European Patent Publication 0,827,029, European Patent Publication 0,827,030, European Patent Publication 0,827,026 European Patent Publication 0,827,031, European Patent Publication 0,827,033, and European Patent Publication 0,827,032, the disclosures of each of which are totally incorporated herein by reference.

Examples of suitable "P" groups include (but are not limited to) unsaturated ester groups, such as acryloyl groups, methacryloyl groups, glycidyl methacryloyl groups, cinnamoyl groups, crotonoyl groups, ethacryloyl groups, oleoyl groups, linoleoyl groups, maleoyl groups, fumaroyl groups, itaconoyl groups, citraconoyl groups, phenylmaleoyl groups, esters of 3-hexene-1,6-dicarboxylic acid, and the like, with an example illustrated below for acryloyl groups,



wherein a, b, c, and d are each integers of 0, 1, 2, 3, or 4, provided that at least one of a, b, c, and d is equal to or greater than 1 in at least some of the monomer repeat units of the polymer, and n is an integer representing the number of repeating monomer units, ether groups, of the above formula wherein the



groups shown above are replaced with, for example,



groups, wherein R is an alkyl group, preferably with from 1 to about 30 carbon atoms, more preferably with from 1 to about 15 carbon atoms, and most preferably with 1 carbon atom, alkylcarboxymethylene groups, of the above formula wherein the



groups shown above are replaced with, for example,



groups, wherein R is an alkyl group (including saturated, unsaturated, and cyclic alkyl groups), preferably with from

1 to about 30 carbon atoms, more preferably with from 1 to about 6 carbon atoms, a substituted alkyl group, an aryl group, preferably with from 6 to about 30 carbon atoms, more preferably with from 1 to about 2 carbon atoms, a substituted aryl group, an arylalkyl group, preferably with from 7 to about 35 carbon atoms, more preferably with from 7 to about 15 carbon atoms, or a substituted arylalkyl group, wherein the substituents on the substituted alkyl, aryl, and arylalkyl groups can be (but are not limited to) alkoxy groups, preferably with from 1 to about 6 carbon atoms, aryloxy groups, preferably with from 6 to about 24 carbon atoms, arylalkyloxy groups, preferably with from 7 to about 30 carbon atoms, hydroxy groups, amine groups, imine groups, ammonium groups, pyridine groups, pyridinium groups, ether groups, ester groups, amide groups, carbonyl groups, thiocarbonyl groups, sulfate groups, sulfonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein two or more substituents can be joined together to form a ring, epoxy groups, of the above formula wherein the



groups shown above are replaced with, for example,



45 groups, allyl groups, vinyl groups, and unsaturated ether groups, of the above formula wherein the



groups shown above are replaced with, for example,



groups, unsaturated ammonium groups and unsaturated phosphonium groups, of the above formula wherein the



groups shown above are replaced with, for example,



groups or similar phosphonium groups, hydroxyalkyl groups, illustrated below for an example with hydroxy methyl groups



wherein a, b, c, and d are each integers of 0, 1, 2, 3, or 4, provided that at least one of a, b, c, and d is equal to or greater than 1 in at least some of the monomer repeat units of the polymer, and n is an integer representing the number of repeating monomer units, and the like. Under certain conditions, such as imaging with electron beam, deep ultraviolet, or x-ray radiation, polymers having haloalkyl groups (with halomethyl groups being preferred), of the general formula



wherein n is an integer of 1, 2, 3, 4, or 5, R is an alkyl group, including both saturated, unsaturated, linear, branched, and cyclic alkyl groups, preferably with from 1 to about 11 carbon atoms, more preferably with from 1 to about 5 carbon atoms, even more preferably with from 1 to about 3 carbon atoms, and most preferably with 1 carbon atom, or a substituted alkyl group, an arylalkyl group, preferably with from 7 to about 29 carbon atoms, more preferably with from 7 to about 17 carbon atoms, even more preferably with from 7 to about 13 carbon atoms, and most preferably with from 7 to about 9 carbon atoms, or a substituted arylalkyl group, and X is a halogen atom, such as fluorine, chlorine, bromine, or iodine, a, b, c, and d are each integers of 0, 1, 2, 3, or 4, provided that at least one of a, b, c, and d is equal to or greater than 1 in at least some of the monomer repeat units of the polymer, and n is an integer representing the number of repeating monomer units, are also photoactive.

The degree of substitution of the polymer with the photosensitivity-imparting substituents (i.e., the average number of photosensitivity-imparting substituents per monomer repeat unit) preferably is from about 0.25 to about 1.2, and more preferably from about 0.65 to about 0.8,

although the degree of substitution can be outside these ranges. This degree of substitution generally corresponds to from about 0.5 to about 1.3 milliequivalents of photosensitivity-imparting substituent per gram of resin.

5 In another embodiment, the polymer of the above formula is substituted with two different functional groups, one of which imparts photosensitivity to the polymer and one of which imparts water solubility or water dispersability to the polymer. Examples of reactants which can be reacted with 10 the polymer to substitute the polymer with suitable water solubility enhancing groups or water dispersability enhancing groups include tertiary amines, of the general formula



20 which add to the polymer quaternary ammonium groups, of the general formula



30 wherein R<sub>1</sub>, R<sub>2</sub>, and R<sub>3</sub> each, independently of the others, can be (but are not limited to) alkyl groups, typically with from 1 to about 30 carbon atoms, substituted alkyl groups, aryl groups, typically with from 6 to about 18 carbon atoms, substituted aryl groups, arylalkyl groups, typically with from 7 to about 19 carbon atoms, and substituted arylalkyl groups, and X represents a halogen atom, such as fluorine, chlorine, bromine, or iodine; tertiary phosphines, of the general formula



40 which add to the polymer quaternary phosphonium groups of the general formula



50 wherein R<sub>1</sub>, R<sub>2</sub>, and R<sub>3</sub> each, independently of the others, can be (but are not limited to) alkyl groups, typically with from 1 to about 30 carbon atoms, substituted alkyl groups, aryl groups, typically with from 6 to about 18 carbon atoms, substituted aryl groups, arylalkyl groups, typically with from 7 to about 19 carbon atoms, and substituted arylalkyl groups, and X represents a halogen atom, such as fluorine, chlorine, bromine, or iodine; alkyl thio ethers, of the general formula



55 which add to the polymer sulfonium groups of the general formula



wherein  $R_1$  and  $R_2$  each, independently of the other, can be (but are not limited to) alkyl groups, typically with from 1 to about 6 carbon atoms and preferably with 1 carbon atom, and substituted alkyl groups, and  $X$  represents a halogen atom, such as fluorine, chlorine, bromine, or iodine; wherein the substituents on the substituted alkyl, aryl, and arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein two or more substituents can be joined together to form a ring. The degree of substitution (i.e., the average number of water solubility imparting groups or water dispersability imparting groups per monomer repeat unit) typically is from about 0.25 to about 4.0, and preferably from about 0.5 to about 2, although the degree of substitution can be outside these ranges. Optimum amounts of substitution are from about 0.8 to about 2 milliequivalents of water solubility imparting group or water dispersability imparting group per gram of resin, and preferably from about 1 to about 1.5 milliequivalents of water solubility imparting group or water dispersability imparting group per gram of resin.

In one specific embodiment, the photopatternable polymer has both haloalkyl substituents, such as chloromethyl groups, bromomethyl groups, or the like, and other photosensitivity-imparting groups, such as unsaturated ester groups, including acryloyl groups, methacryloyl groups, or the like, and is illustrated below for the embodiment with chloromethyl groups and acryloyl groups:

$n$  is an integer representing the number of repeating monomer units. In this instance, the polymer typically has a degree of substitution of from about 0.25 to about 2.25, preferably from about 0.75 to about 2, and more preferably from about 0.75 to about 1 halomethyl group per monomer repeat unit, and from about 0.25 to about 1.5, preferably from about 0.5 to about 0.8, and more preferably about 0.75 of the other photosensitivity-imparting groups per monomer repeat unit, although the relative amounts can be outside these ranges.

Blends of polymers can also be employed, provided that at least one of the polymers contains photosensitivity-imparting substituents. Blends of polymers preferably contain at least 25 percent by weight of the polymer having photosensitivity-imparting substituents.

Specific embodiments of the invention will now be described in detail. These examples are intended to be illustrative, and the invention is not limited to the materials, conditions, or process parameters set forth in these embodiments. All parts and percentages are by weight unless otherwise indicated.

#### POLYMER SYNTHESIS EXAMPLE I

A polyarylene ether ketone of the formula



wherein  $n$  is between about 6 and about 30 (hereinafter referred to as poly(4-CPK-BPA)) was prepared as follows. A 35 1 liter, 3-neck round-bottom flask equipped with a Dean-Stark (Barrett) trap, condenser, mechanical stirrer, argon inlet, and stopper was situated in a silicone oil bath. 4,4'-Dichlorobenzophenone (Aldrich 11,370, Aldrich Chemical Co., Milwaukee, Wis., 50 grams), bis-phenol A 40 (Aldrich 23,965-8, 48.96 grams), potassium carbonate (65.56 grams), anhydrous N,N-dimethylacetamide (300 milliliters), and toluene (55 milliliters) were added to the



wherein  $e$ ,  $f$ ,  $g$ ,  $h$ ,  $i$ ,  $j$ ,  $k$ , and  $m$  are each integers of 0, 1, 2, 3, or 4, provided that the sum of  $i+e$  is no greater than 4, the sum of  $j+f$  is no greater than 4, the sum of  $k+g$  is no greater than 4, and the sum of  $m+h$  is no greater than 4, and provided that at least one of  $e$ ,  $f$ ,  $g$ , and  $h$  is equal to at least 1 in at least some of the monomer repeat units of the polymer, and

flask and heated to 175° C. (oil bath temperature) while the volatile toluene component was collected and removed. After 24 hours of heating at 175° C. with continuous stirring, an aliquot of the reaction product that had been precipitated into methanol was analyzed by gel permeation chromatography (gpc) (elution solvent was tetrahydrofuran) with the

45

following results:  $M_n$  4464,  $M_{peak}$  7583,  $M_w$  7927,  $M_z$  12,331, and  $M_{z+1}$  16,980. After 48 hours at 175° C. with continuous stirring, the reaction mixture was filtered to remove potassium carbonate and precipitated into methanol (2 gallons). The polymer (poly(4-CPK-BPA)) was isolated in 86% yield after filtration and drying in vacuo. GPC analysis was as follows:  $M_n$  5347,  $M_{peak}$  16,126,  $M_w$  15,596,  $M_z$  29,209, and  $M_{z+1}$  42,710. The glass transition temperature of the polymer was about 120±10° C. as determined using differential scanning calorimetry at a heating rate of 20° C. per minute. As a result of the stoichiometries used in the reaction, it is believed that this polymer had end groups derived from bis-phenol A.

## POLYMER SYNTHESIS EXAMPLE II

A polyarylene ether ketone of the formula



wherein n is between about 2 and about 30 (hereinafter referred to as poly(4-CPK-BPA)) was prepared as follows. A 5 liter, 3-neck round-bottom flask equipped with a Dean-Stark (Barrett) trap, condenser, mechanical stirrer, argon inlet, and stopper was situated in a silicone oil bath. 4,4'-Dichlorobenzophenone (Aldrich 11,370, Aldrich Chemical Co., Milwaukee, Wis., 250 grams), bis-phenol A (Aldrich 23,965-8, 244.8 grams), potassium carbonate (327.8 grams), anhydrous N,N-dimethylacetamide (1,500 milliliters), and toluene (275 milliliters) were added to the flask and heated to 175° C. (oil bath temperature) while the volatile toluene component was collected and removed. After 48 hours of heating at 175° C. with continuous stirring, the reaction mixture was filtered to remove insoluble salts, and the resultant solution was added to methanol (5 gallons) to precipitate the polymer. The polymer was isolated by filtration, and the wet filter cake was washed with water (3 gallons) and then with methanol (3 gallons). The yield was 360 grams of vacuum dried product. The molecular weight of the polymer was determined by gel permeation chromatography (gpc) (elution solvent was tetrahydrofuran) with the following results:  $M_n$  3,601,  $M_{peak}$  5,377,  $M_w$  4,311,  $M_z$  8,702, and  $M_{z+1}$  12,951. The glass transition temperature of the polymer was between 125 and 155° C. as determined using differential scanning calorimetry at a heating rate of 20° C. per minute dependent on molecular weight. As a result of the stoichiometries used in the reaction, it is believed that this polymer had end groups derived from bis-phenol A.

## POLYMER SYNTHESIS EXAMPLE III

Poly(4-CPK-BPA) prepared as described in Polymer synthesis Example I (10 grams) in 1,1,2,2-tetrachloroethane (100 milliliters, 161.9 grams), paraformaldehyde (5 grams), p-toluenesulfonic acid monohydrate (1 gram), acrylic acid (15.8 grams), and crushed 4-methoxy-phenol (MEHQ, 0.2 gram) were charged in a 6.5 fluid ounce beverage bottle equipped with a magnetic stirrer. The bottle was stoppered with a rubber septum and was then heated to 105° C. in a silicone oil bath under argon using a needle inlet. The argon needle inlet was removed when the oil bath achieved 90° C. Heating at 105° C. was continued with constant magnetic

46

stirring for 1.5 hours. More MEHQ (0.2 grams) in 1 milliliter of 1,1,2,2-tetrachloroethane was then added by syringe, and heating at 105° C. with stirring was continued for 1.5 hours longer. The reaction mixture was initially a cloudy suspension which became clear on heating. The reaction vessel was immersed as much as possible in the hot oil bath to prevent condensation of paraformaldehyde onto cooler surfaces of the reaction vessel. The reaction mixture was allowed to return to 25° C. and was then filtered through a 25 to 50 micron sintered glass Buchner funnel. The reaction solution was added to methanol (1 gallon) to precipitate the polymer designated poly(acryloylmethyl-4-CPK-BPA), of the formula



wherein n is between about 6 and about 50.  $^1\text{H}$  NMR spectrometry was used to identify approximately 1 acryloylmethyl group for every four monomer (4-CPK-BPA) repeat units (i.e., a degree of acryloylation of 0.25). The poly(acryloylmethyl-4-CPK-BPA) was then dissolved in methylene chloride and reprecipitated into methanol (1 gallon) to yield 10 grams of fluffy white solid.

## POLYMER SYNTHESIS EXAMPLE IV

A solution of chloromethyl ether in methyl acetate was made by adding 282.68 grams (256 milliliters) of acetyl chloride to a mixture of dimethoxy methane (313.6 grams, 366.8 milliliters) and methanol (10 milliliters) in a 5 liter 3-neck round-bottom flask equipped with a mechanical stirrer, argon inlet, reflux condenser, and addition funnel. The solution was diluted with 1,066.8 milliliters of 1,1,2,2-tetrachloroethane and then tin tetrachloride (2.4 milliliters) was added via a gas-tight syringe along with 1,1,2,2-tetrachloroethane (133.2 milliliters) using an addition funnel. The reaction solution was heated to 500° C. Thereafter, a solution of poly(4-CPK-BPA) prepared as described in Polymer Synthesis Example II (160.8 grams) in 1,000 milliliters of tetrachloroethane was added rapidly. The reaction mixture was then heated to reflux with an oil bath set at 110° C. After four hours reflux with continuous stirring, heating was discontinued and the mixture was allowed to cool to 25° C. The reaction mixture was transferred in stages to a 2 liter round bottom flask and concentrated using a rotary evaporator with gentle heating up to 50° C. while reduced pressure was maintained with a vacuum pump trapped with liquid nitrogen. The concentrate was added to methanol (4 gallons) to precipitate the polymer using a Waring blender. The polymer was isolated by filtration and vacuum dried to yield 200 grams of poly(4-CPK-BPA) with 1.5 chloromethyl groups per repeat unit as identified using  $^1\text{H}$  NMR spectroscopy. When the same reaction was carried out for 1, 2, 3, and 4 hours, the amount of chloromethyl groups per repeat unit was 0.76, 1.09, 1.294, and 1.496, respectively.

Solvent free polymer was obtained by reprecipitation of the polymer (75 grams) in methylene chloride (500 grams)

47

into methanol (3 gallons) followed by filtration and vacuum drying to yield 70.5 grams (99.6% theoretical yield) of solvent free polymer.

When the reaction was carried out under similar conditions except that 80.4 grams of poly(4-CPK-BPA) was used instead of 160.8 grams and the amounts of the other reagents were the same as indicated above, the polymer is formed with 1.31, 1.50, 1.75, and 2 chloromethyl groups per repeat unit in 1, 2, 3, and 4 hours, respectively, at 110° C. (oil bath temperature).

When 241.2 grams of poly(4-CPK-BPA) was used instead of 160.8 grams with the other reagents fixed, poly(4-CPK-BPA) was formed with 0.79, 0.90, 0.98, 1.06, 1.22, and 1.38 chloromethyl groups per repeat unit in 1, 2, 3, 4, 5, and 6 hours, respectively, at 110° C. (oil bath temperature).

When 321.6 grams of poly(4-CPK-BPA) was used instead of 160.8 grams with the other reagents fixed, poly(4-CPK-BPA) was formed with 0.53, 0.59, 0.64, 0.67, 0.77, 0.86, 0.90, and 0.97 chloromethyl groups per repeat unit in 1, 2, 3, 4, 5, 6, 7, and 8 hours, respectively, at 110° C. (oil bath temperature).

#### POLYMER SYNTHESIS EXAMPLE V

A polyarylene ether ketone of the formula



was prepared as described in Polymer Synthesis Example I. A solution of chloromethyl ether in methyl acetate was made by adding 35.3 grams of acetyl chloride to a mixture of dimethoxy methane (45 milliliters) and methanol (1.25 milliliters) in a 500 milliliter 3-neck round-bottom flask equipped with a mechanical stirrer, argon inlet, reflux condenser, and addition funnel. The solution was diluted with 150 milliliters of 1,1,2,2-tetrachloroethane and then tin tetrachloride (0.3 milliliters) was added via syringe. The solution was heated to reflux with an oil bath set at 110° C. Thereafter, a solution of poly(4-CPK-BPA) (10 grams) in 125 milliliters of 1,1,2,2-tetrachloroethane was added over 8 minutes. After two hours reflux with continuous stirring, heating was discontinued and the mixture was allowed to cool to 25° C. The reaction mixture was transferred to a rotary evaporator with gentle heating at between 50 and 55° C. After 1 hour, when most of the volatiles had been removed, the reaction mixture was added to methanol (each 25 milliliters of solution was added to 0.75 liter of methanol) to precipitate the polymer using a Waring blender. The precipitated polymer was collected by filtration, washed with methanol, and air-dried to yield 13 grams of off-white powder. The polymer had about 1.5 CH<sub>2</sub>Cl groups per repeat unit.

#### POLYMER SYNTHESIS EXAMPLE VI

A solution was prepared containing 90 grams of a chloromethylated polymer prepared as described in Polymer Synthesis Example IV with 1.5 chloromethyl groups per repeat unit in 639 milliliters (558.5 grams) of N,N-dimethylacetamide and the solution was magnetically stirred at 25° C. with sodium acrylate (51.39 grams) for 1 week. The reaction mixture was then centrifuged, and the super-

48

nate was added to methanol (4.8 gallons) using a Waring blender in relative amounts of 25 milliliters of polymer solution per 0.75 liter of methanol. The white powder that precipitated was filtered, and the wet filter cake was washed with water (3 gallons) and then methanol (3 gallons). The polymer was then isolated by filtration and vacuum dried to yield 73.3 grams of a white powder. The polymer had 3 acrylate groups for every 4 repeating monomer units and 3 chloromethyl groups for every 4 repeating monomer units and a weight average molecular weight of about 25,000.

When the reaction was repeated with poly(4-CPK-BPA) with 2 chloromethyl groups per repeat unit and the other reagents remained the same, the reaction took four days to achieve 0.76 acrylate groups per repeat unit and 1.24 chloromethyl groups per repeat unit.

When the reaction was repeated with poly(4-CPK-BPA) with 1.0 chloromethyl groups per repeat unit and the other reagents remained the same, the reaction took 14-days to achieve 0.75 acrylate groups per repeat unit and 2.5 chloromethyl groups per repeat unit.

#### POLYMER SYNTHESIS EXAMPLE VII

A chloromethylated polyarylene ether ketone having 1.5 chloromethyl groups per repeat unit was prepared as described in Polymer Synthesis Example IV. A solution containing 10 grams of the chloromethylated polymer in 71 milliliters of N,N-dimethyl acetamide was magnetically stirred with 5.71 grams of sodium acetate (obtained from Aldrich Chemical Co., Milwaukee, Wis.). The reaction was allowed to proceed for one week. The reaction mixture was then centrifuged and the supernate was added to methanol (0.5 gallon) to precipitate the polymer. The polymer was then filtered, washed with water (2 liters), and subsequently washed with methanol (0.5 gallon). Approximately half of the chloromethyl groups were replaced with methylcarboxymethylene groups, and it is believed that the polymer was of the formula



When the process was repeated under similar conditions but allowed to proceed for about 2 weeks, nearly all of the chloromethyl groups were replaced with methylcarboxymethylene groups, and the resulting polymer was believed to be of the formula

49



## POLYMER SYNTHESIS EXAMPLE VIII

The process of Polymer Synthesis Example VII was repeated except that the 5.71 grams of sodium acetate were replaced with 5.71 grams of sodium methoxide (obtained from Aldrich Chemical Co., Milwaukee, Wis.). After about two hours, approximately half of the chlorine atoms on the chloromethyl groups were replaced with methoxy groups, and it is believed that the polymer was of the formula



When the process was repeated under similar conditions but allowed to proceed for about 2 weeks, nearly all of the chlorine atoms on the chloromethyl groups were replaced with methoxy groups, and the resulting polymer was believed to be of the formula



## POLYMER SYNTHESIS EXAMPLE IX

A chloromethylated polyarylene ether ketone was prepared as described in Polymer Synthesis Example V. A solution was then prepared containing 11 grams of the chloromethylated polymer in 100 milliliters (87.4 grams) of N,N-dimethylacetamide and the solution was magnetically stirred at 25° C. with sodium acrylate (30 grams) for 1 week. The reaction mixture was then filtered and added to methanol using a Waring blender in relative amounts of 25 milliliters of polymer solution per 0.75 liter of methanol. The white powder that precipitated was reprecipitated into methanol from a 20 weight percent solids solution in methylene chloride and was then air dried to yield 7.73 grams of a white powder. The polymer had 3 acrylate groups for every 4 repeating monomer units and 3 chloromethyl groups for every 4 repeating monomer units.

50

## POLYMER SYNTHESIS EXAMPLE X

A polyarylene ether ketone of the formula



wherein n is between about 6 and about 30 (hereinafter referred to as poly(4-CPK-BPA)) was prepared as follows. A 1 liter, 3-neck round-bottom flask equipped with a Dean-Stark (Barrett) trap, condenser, mechanical stirrer, argon inlet, and stopper was situated in a silicone oil bath. 4,4'-Dichlorobenzophenone (Aldrich 11,370, Aldrich Chemical Co., Milwaukee, Wis., 53.90 grams), bis-phenol A (Aldrich 23,965-8, 45.42 grams), potassium carbonate (65.56 grams), anhydrous N,N-dimethylacetamide (300 milliliters), and toluene (55 milliliters) were added to the flask and heated to 175° C. (oil bath temperature) while the volatile toluene component was collected and removed. After 24 hours of heating at 175° C. with continuous stirring, the reaction mixture was filtered to remove potassium carbonate and precipitated into methanol (2 gallons). The polymer (poly(4-CPK-BPA)) was isolated in 86% yield after filtration and drying in vacuo. GPC analysis was as follows:  $M_n$  4,239,  $M_{peak}$  9,164,  $M_w$  10,238,  $M_z$  18,195, and  $M_{z+1}$  25,916. Solution cast films from methylene chloride were clear, tough, and flexible. As a result of the stoichiometries used in the reaction, it is believed that this polymer had end groups derived from 4,4-dichlorobenzophenone.

## POLYMER SYNTHESIS EXAMPLE XI

A benzophenone-terminated polyarylene ether ketone prepared as described in Polymer Synthesis Example X was chloromethyl substituted as described in Polymer Synthesis Example IV, resulting in a benzophenone-terminated, chloromethylated polymer having 0.5 chloromethyl groups per repeat unit.

A solution was prepared containing the benzophenone-terminated chloromethylated polyarylene ether ketone thus prepared in N-methylpyrrolidinone at a concentration of 33.7 percent by weight polymer solids. To this solution was added N,N-dimethyl ethyl methacrylate (obtained from Aldrich Chemical Co., Milwaukee, Wis.) in an amount of 6.21 percent by weight of the polymer solution, and the resulting solution was stirred for 2 hours. The reaction of the chloromethyl groups with the N,N-dimethyl ethyl methacrylate occurred quickly, resulting in formation of a polymer having about 0.5 N,N-dimethyl ethyl methacrylate groups per monomer repeat unit.

## POLYMER SYNTHESIS EXAMPLE XII

Fifty grams of a polymer having 0.75 acrylate groups per repeat unit and 0.75 chloromethyl groups per repeat unit prepared as described in Polymer Synthesis Example VI is dissolved in 117 milliliters of N,N-dimethylacetamide and magnetically stirred at 5° C. in an ice bath with 30 milliliters of trimethylamine. The reaction mixture is allowed to return to 25° C. over two hours and stirring is continued for an additional two hours. The unreacted trimethylamine is then removed using a rotary evaporator and the resulting polymer has both acrylate substituents and trimethylammonium chloride substituents.

51

## POLYMER SYNTHESIS EXAMPLE XIII

A polymer of the formula



wherein n represents the number of repeating monomer units was prepared as follows. A 500 milliliter, 3-neck round-bottom flask equipped with a Dean-Stark (Barrett) trap, condenser, mechanical stirrer, argon inlet, and stopper was situated in a silicone oil bath. 4,4'-Dichlorobenzophenone (Aldrich 11,370, Aldrich Chemical Co., Milwaukee, Wis., 16.32 grams, 0.065 mol), bis(4-hydroxyphenyl)methane (Aldrich, 14.02 grams, 0.07 mol), potassium carbonate (21.41 grams), anhydrous N,N-dimethylacetamide (100 milliliters), and toluene (100 milliliters) were added to the flask and heated to 175° C. (oil bath temperature) while the volatile toluene component was collected and removed. After 48 hours of heating at 175° C. with continuous stirring, the reaction mixture was filtered and added to methanol to precipitate the polymer, which was collected by filtration, washed with water, and then washed with methanol. The yield of vacuum dried product, poly(4-CPK-BPM), was 24 grams. The polymer dissolved on heating in N-methylpyrrolidinone, N,N-dimethylacetamide, and 1,1,2,2-tetrachloroethane. The polymer remained soluble after the solution had cooled to 25° C.

## POLYMER SYNTHESIS EXAMPLE XIV

The polymer poly(4-CPK-BPM), prepared as described in Polymer Synthesis Example XIII, was acryloylated with paraformaldehyde by the process described in Polymer Synthesis Example II. Similar results were obtained.

## POLYMER SYNTHESIS EXAMPLE XV

The polymer poly(4-CPK-BPM), prepared as described in Polymer Synthesis Example XIII, was chloromethylated as follows. A solution of chloromethyl methyl ether (6 mmol/milliliter) in methyl acetate was prepared by adding acetyl chloride (35.3 grams) to a mixture of dimethoxymethane (45 milliliters) and methanol (1.25 milliliters). The solution was diluted with 150 milliliters of 1,1,2,2-tetrachloroethane and then tin tetrachloride (0.3 milliliters) was added. After taking the mixture to reflux using an oil bath set at 110° C., a solution of poly(4-CPK-BPM) (10 grams) in 125 milliliters of 1,1,2,2-tetrachloroethane was added. Reflux was maintained for 2 hours and then 5 milliliters of methanol were added to quench the reaction. The reaction solution was added to 1 gallon of methanol using a Waring blender to precipitate the product, chloromethylated poly(4-CPK-BPM), which was collected by filtration and vacuum dried. The yield was 9.46 grams of poly(4-CPK-BPM) with 2 chloromethyl groups per polymer repeat unit. The polymer had the following structure:

52



## POLYMER SYNTHESIS EXAMPLE XVI

Poly(4-CPK-BPM) with 2 chloromethyl groups per repeat unit (1 gram, prepared as described in Polymer Synthesis Example XV) in 20 milliliters of N,N-dimethylacetamide was magnetically stirred with sodium acrylate for 112 hours at 25° C. The solution was added to methanol using a Waring blender to precipitate the polymer, which was filtered and vacuum dried. Between 58 and 69 percent of the chloromethyl groups had been replaced with acryloyl groups. The product had the following formula:



## POLYMER SYNTHESIS EXAMPLE XVII

A polymer of the formula



wherein n represents the number of repeating monomer units was prepared as follows. A 500 milliliter, 3-neck round-bottom flask equipped with a Dean-Stark (Barrett) trap, condenser, mechanical stirrer, argon inlet, and stopper was situated in a silicone oil bath. 4,4'-Dichlorobenzophenone (Aldrich 11,370, Aldrich Chemical Co., Milwaukee, Wis., 16.32 grams, 0.065 mol), hexafluorobisphenol A (Aldrich, 23.52 grams, 0.07 mol), potassium carbonate (21.41 grams), anhydrous N,N-dimethylacetamide (100 milliliters), and toluene (100 milliliters) were added to the flask and heated to 175° C. (oil bath temperature) while the volatile toluene component was collected and removed. After 48 hours of heating at 175° C. with continuous stirring, the reaction mixture was filtered and added to methanol to precipitate the polymer, which was collected by filtration, washed with water, and then washed with methanol. The yield of vacuum dried product, poly(4-CPK-HFBPA), was 20 grams. The polymer was analyzed by gel permeation chromatography (gpc) (elution solvent was tetrahydrofuran) with the following results:  $M_n$  1,975,  $M_{peak}$  2,281,  $M_w$  3,588, and  $M_{z+1}$  8,918.

## POLYMER SYNTHESIS EXAMPLE XVIII

The polymer poly(4-CPK-HFBPA), prepared as described in Polymer Synthesis Example XVII, was acryloylated with

53

paraformaldehyde by the process described in Polymer Synthesis Example II. Similar results were obtained.

## POLYMER SYNTHESIS EXAMPLE XIX

The polymer poly(4-CPK-HFBPA), prepared as described in Polymer Synthesis Example XVII, is chloromethylated by the process described in Polymer Synthesis Example XV. It is believed that similar results will be obtained.

## POLYMER SYNTHESIS EXAMPLE XX

The chloromethylated polymer poly(4-CPK-HFBPA), prepared as described in Polymer Synthesis Example XIX, is acryloylated by the process described in Polymer Synthesis Example XVI. It is believed that similar results will be obtained.

## POLYMER SYNTHESIS EXAMPLE XXI

A polymer of the formula



wherein n represents the number of repeating monomer units was prepared as follows. A 1-liter, 3-neck round-bottom flask equipped with a Dean-Stark (Barrett) trap, condenser, mechanical stirrer, argon inlet, and stopper was situated in a silicone oil bath. 4,4'-Difluorobenzophenone (Aldrich Chemical Co., Milwaukee, Wis., 43.47 grams, 0.1992 mol), 9,9'-bis(4-hydroxyphenyl)fluorenone (Ken Seika, Rumson, N.J., 75.06 grams, 0.2145 mol), potassium carbonate (65.56 grams), anhydrous N,N-dimethylacetamide (300 milliliters), and toluene (52 milliliters) were added to the flask and heated to 175° C. (oil bath temperature) while the volatile toluene component was collected and removed. After 5 hours of heating at 175° C. with continuous stirring, the reaction mixture was allowed to cool to 25° C. The solidified mass was treated with acetic acid (vinegar) and extracted with methylene chloride, filtered, and added to methanol to precipitate the polymer, which was collected by filtration, washed with water, and then washed with methanol. The yield of vacuum dried product, poly(4-CPK-FBP), was 71.7 grams. The polymer was analyzed by gel permeation chromatography (gpc) (elution solvent was tetrahydrofuran) with the following results:  $M_n$  59,100,  $M_{peak}$  144,000,  $M_w$  136,100,  $M_z$  211,350, and  $M_{z+1}$  286,100.

## POLYMER SYNTHESIS EXAMPLE XXII

A polymer of the formula



wherein n represents the number of repeating monomer units was prepared as follows. A 1-liter, 3-neck round-bottom

54

flask equipped with a Dean-Stark (Barrett) trap, condenser, mechanical stirrer, argon inlet, and stopper was situated in a silicone oil bath. 4,4'-Dichlorobenzophenone (Aldrich Chemical Co., Milwaukee, Wis., 50.02 grams, 0.1992 mol), 9,9'-bis(4-hydroxyphenyl)fluorenone (Ken Seika, Rumson, N.J., 75.04 grams, 0.2145 mol), potassium carbonate (65.56 grams), anhydrous N,N-dimethylacetamide (300 milliliters), and toluene (52 milliliters) were added to the flask and heated to 175° C. (oil bath temperature) while the volatile toluene component was collected and removed. After 24 hours of heating at 175° C. with continuous stirring, the reaction mixture was allowed to cool to 25° C. The reaction mixture was filtered and added to methanol to precipitate the polymer, which was collected by filtration, washed with water, and then washed with methanol. The yield of vacuum dried product, poly(4-CPK-FBP), was 60 grams.

## POLYMER SYNTHESIS EXAMPLE XXIII

The polymer poly(4-CPK-FBP), prepared as described in Polymer Synthesis Example XXII, was chloromethylated as follows. A solution of chloromethyl methyl ether (6 mmol/25 milliliter) in methyl acetate was prepared by adding acetyl chloride (38.8 grams) to a mixture of dimethoxymethane (45 milliliters) and methanol (1.25 milliliters). The solution was diluted with 100 milliliters of 1,1,2,2-tetrachloroethane and then tin tetrachloride (0.5 milliliters) was added in 50 milliliters of 1,1,2,2-tetrachloroethane. After taking the mixture to reflux using an oil bath set at 100° C., a solution of poly(4-CPK-FBP) (10 grams) in 125 milliliters of 1,1,2,2-tetrachloroethane was added. The reaction temperature was maintained at 100° C. for 1 hour and then 5 milliliters of methanol were added to quench the reaction. The reaction solution was added to 1 gallon of methanol using a Waring blender to precipitate the product, chloromethylated poly(4-CPK-FBP), which was collected by filtration and vacuum dried. The yield was 9.5 grams of poly(4-CPK-FBP) with 1.5 chloromethyl groups per polymer repeat unit. When the reaction was carried out at 110° C. (oil bath set temperature), the polymer gelled within 80 minutes. The polymer had the following structure:



## POLYMER SYNTHESIS EXAMPLE XXIV

Poly(4-CPK-FBP) with 1.5 chloromethyl groups per repeat unit (1 gram, prepared as described in Polymer Synthesis Example XXIII) in 20 milliliters of N,N-dimethylacetamide was magnetically stirred with sodium acrylate for 112 hours at 25° C. The solution was added to methanol using a Waring blender to precipitate the polymer, which was filtered and vacuum dried. About 50 percent of the chloromethyl groups had been replaced with acryloyl groups. The product had the following formula:



## POLYMER SYNTHESIS EXAMPLE XXV

A polymer of the formula



wherein n represents the number of repeating monomer units was prepared as follows. A 1-liter, 3-neck round-bottom flask equipped with a Dean-Stark (Barrett) trap, condenser, mechanical stirrer, argon inlet, and stopper was situated in a silicone oil bath. 4,4'-Difluorobenzophenone (Aldrich Chemical Co., Milwaukee, Wis., 16.59 grams), bisphenol A (Aldrich 14.18 grams, 0.065 mol), potassium carbonate (21.6 grams), anhydrous N,N-dimethylacetamide (100 milliliters), and toluene (30 milliliters) were added to the flask and heated to 175° C. (oil bath temperature) while the volatile toluene component was collected and removed. After 4 hours of heating at 175° C. with continuous stirring, the reaction mixture was allowed to cool to 25° C. The solidified mass was treated with acetic acid (vinegar) and extracted with methylene chloride, filtered, and added to methanol to precipitate the polymer, which was collected by filtration, washed with water, and then washed with methanol. The yield of vacuum dried product, poly(4-FPK-BPA), was 12.22 grams. The polymer was analyzed by gel permeation chromatography (gpc) (elution solvent was tetrahydrofuran) with the following results:  $M_n$  5,158,  $M_{peak}$  15,080,  $M_w$  17,260, and  $M_{z+1}$  39,287. To obtain a lower molecular weight, the reaction can be repeated with a 15 mol % offset in stoichiometry.

## POLYMER SYNTHESIS EXAMPLE XXVI

A polymer of the formula



wherein n represents the number of repeating monomer units was prepared as follows. A 250 milliliter, 3-neck round-

bottom flask equipped with a Dean-Stark (Barrett) trap, condenser, mechanical stirrer, argon inlet, and stopper was situated in a silicone oil bath. 4'-Methylbenzoyl-2,4-dichlorobenzene (0.0325 mol, 8.6125 grams), bis-phenol A (Aldrich 23,965-8, 0.035 mol, 7.99 grams), potassium carbonate (10.7 grams), anhydrous N,N-dimethylacetamide (60 milliliters), and toluene (60 milliliters, 49.1 grams) were added to the flask and heated to 175° C. (oil bath temperature) while the volatile toluene component was collected and removed. After 24 hours of heating at 175° C. with continuous stirring, the reaction product was filtered and the filtrate was added to methanol to precipitate the polymer. The wet polymer cake was isolated by filtration, washed with water, then washed with methanol, and thereafter vacuum dried. The polymer (7.70 grams, 48% yield) was analyzed by gel permeation chromatography (gpc) (elution solvent was tetrahydrofuran) with the following results:  $M_n$  1,898,  $M_{peak}$  2,154,  $M_w$  2,470,  $M_z$  3,220, and  $M_{z+1}$  4,095.

## POLYMER SYNTHESIS EXAMPLE XXVII

A polymer of the formula



wherein n represents the number of repeating monomer units was prepared by repeating the process of Polymer Synthesis Example XXVI except that the 4'-methylbenzoyl-2,4-dichlorobenzene starting material was replaced with 8.16 grams (0.0325 mol) of benzoyl-2,4-dichlorobenzene and the oil bath was heated to 170° C. for 24 hours.

## POLYMER SYNTHESIS EXAMPLE XXVIII

Chloromethylated phenoxy resins, polyethersulfones, and polyphenylene oxides are prepared by reacting the unsubstituted polymers with tin tetrachloride and 1-chloromethoxy-4-chlorobutane as described by W. H. Daly et al. in *Polymer Preprints*, 20(1), 835 (1979), the disclosure of which is totally incorporated herein by reference. The chloromethylation of polyethersulfone and polyphenylene oxide can also be accomplished as described by V. Percec et al. in *Makromol. Chem.*, 185, 2319 (1984), the disclosure of which is totally incorporated herein by reference.

57

Acryloylated polymers are then prepared as follows:



The chloromethylated polymers are acryloylated by allowing the chloromethylated polymer (10 grams) in *N,N*-dimethylacetamide (71 milliliters) to react with acrylic acid sodium salt (5.14 grams) for between 3 and 20 days, depending on the degree of acryloylation desired. Longer reaction times result in increased acrylate functionality.

#### POLYMER SYNTHESIS EXAMPLE XXIX

Poly(4-CPK-BPA) is made with a number average molecular weight of 2,800 as follows. A 5-liter, 3-neck round-bottom flask equipped with a Dean-Stark (Barrett) trap, condenser, mechanical stirrer, argon inlet, and stopper is situated in a silicone oil bath. 4,4'-Dichlorobenzophenone (Aldrich 11,370, Aldrich Chemical Co., Milwaukee, Wis., 250 grams), bis-phenol A (Aldrich 23,965-8, 244.8 grams), potassium carbonate (327.8 grams), anhydrous *N,N*-

58

dimethylacetamide (1,500 milliliters), and toluene (275 milliliters) are added to the flask and heated to 175° C. (oil bath temperature) while the volatile toluene component is collected and removed. After hours of heating 30 hours at 5 175° C. with continuous stirring, the reaction mixture is filtered to remove insoluble salts, and the resultant solution is added to methanol (5 gallons) to precipitate the polymer. The polymer is isolated by filtration, and the wet filter cake is washed with water (3 gallons) and then with methanol (3 10 gallons). The yield is about 360 grams of vacuum dried polymer. It is believed that if the molecular weight of the polymer is determined by gel permeation chromatography (gpc) (elution solvent was tetrahydrofuran) the following results will be obtained:  $M_n$  2,800,  $M_{peak}$  5,800,  $M_w$  6,500, 15  $M_z$  12,000 and  $M_{z+1}$  17,700. As a result of the stoichiometries used in the reaction, it is believed that this polymer has end groups derived from bis-phenol A.

The polymer is then chloromethylated as follows. A solution of chloromethyl ether in methyl acetate is made by 20 adding 282.68 grams (256 milliliters) of acetyl chloride to a mixture of dimethoxy methane (313.6 grams, 366.8 milliliters) and methanol (10 milliliters) in a 5-liter 3-neck round-bottom flask equipped with a mechanical stirrer, argon inlet, reflux condenser, and addition funnel. The 25 solution is diluted with 1,066.8 milliliters of 1,1,2,2-tetrachloroethane and then tin tetrachloride (2.4 milliliters) is added via a gas-tight syringe, along with 1,1,2,2-tetrachloroethane (133.2 milliliters) using an addition funnel. The reaction solution is heated to 50° C. and a solution 30 of poly(4-CPK-BPA) (160.8 grams) in 1,1,2,2-tetrachloroethane (1,000 milliliters) is rapidly added. The reaction mixture is then heated to reflux with an oil bath set at 110° C. After four hours reflux with continuous stirring, heating is discontinued and the mixture is allowed to cool to 35 25° C. The reaction mixture is transferred in stages to a 2 liter round bottom flask and concentrated using a rotary evaporator with gentle heating up to 50° C. and reduced pressure maintained with a vacuum pump trapped with liquid nitrogen. The concentrate is added to methanol (6 40 gallons) to precipitate the polymer using a Waring blender. The polymer is isolated by filtration and vacuum dried to yield 200 grams of poly(4-CPK-BPA) with 1.5 chloromethyl groups per repeat unit. Solvent free polymer is obtained by reprecipitation of the polymer (75 grams) dissolved in 45 methylene chloride (500 grams) into methanol (3 gallons) followed by filtration and vacuum drying to yield 70.5 grams (99.6% yield) of solvent free polymer. To a solution of the chloromethylated poly(4-CPK-BPA) (192 mmol of chloromethyl groups) in 80 milliliters of dioxane is added 12 50 grams (46 mmol) of triphenylphosphine. After 15 hours of reflux with mechanical stirring and cooling to 25° C., the polymer solidifies and the mixture is extracted with diethyl ether using a Waring blender. The yellow product is filtered, washed several times with diethyl ether, and vacuum dried. 55 To a solution of triphenylphosphonium chloride salt of chloromethylated poly(4-CPK-BPA) (14 mmol of phosphonium groups) in 200 milliliters of methanol, 2 milliliters of Triton B (40 weight percent aqueous solution) and 11.5 milliliters (140 mmol) of formaldehyde (37 weight percent aqueous solution) are added. The stirred reaction mixture is 60 treated slowly with 36 milliliters of 50 weight percent aqueous sodium hydroxide. A precipitate starts to appear on addition of the first drops of sodium hydroxide solution. After 10 hours of reaction at 25° C., the precipitate is filtered and vacuum dried. The separated polymer is dissolved in methylene chloride, washed several times with water, and then precipitated with methanol. Alternatively, to a solution 65

59

of solution of 1.8 mmol of phosphonium groups of the triphenylphosphonium chloride salt chloromethylated poly (4-CPK-BPA) in 40 milliliters of methylene chloride at ice-water temperature, 1.6 milliliters (19.5 mmol) of formaldehyde (37 weight percent aqueous solution), and 0.4 milliliters of Triton-B (40 weight percent aqueous solution) is added. The stirred reaction mixture is treated slowly with 5 milliliters (62.5 mmol) of 50 weight percent aqueous sodium hydroxide. After all the hydroxide solution is added, the reaction mixture is allowed to react at 25° C. After 7 hours of reaction, the organic layer is separated, washed with dilute hydrochloric acid, then washed with water, and then precipitated into methanol from chloroform. The polymer has the structure:



Other embodiments and modifications of the present invention may occur to those of ordinary skill in the art subsequent to a review of the information presented herein; these embodiments and modifications, as well as equivalents thereof, are also included within the scope of this invention.

What is claimed is:

1. An ink jet printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, the upper and lower substrates being aligned, mated, and bonded together to form the printhead with the grooves in the upper substrate being aligned with the heating elements in the lower substrate to form droplet emitting nozzles, said upper substrate comprising a material formed by crosslinking or chain extending a polymer of the formula



60

-continued

III



wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of the monomer repeat units of the polymer. A is



or mixtures thereof. B is



61

-continued



wherein  $v$  is an integer of from 1 to about 20,



wherein z is an integer of from 2 to about 20,



62

wherein  $u$  is an integer of from 1 to about 20,



wherein w is an integer of from 1 to about 20,



55 or mixtures thereof, and  $n$  is an integer representing the number of repeating monomer units.

2. An ink jet printhead according to claim 1 wherein the insulative layer of the lower substrate comprises a material formed by crosslinking or chain extending a polymer of formula I or II.

3. An ink jet printhead according to claim 2 wherein the printhead is substantially free of an interface between the upper substrate and the insulative layer of the lower substrate.

65 4. An ink jet printhead according to claim 1 wherein the upper substrate is bonded to the insulative layer of the lower substrate with an adhesive which comprises a material

63

formed by crosslinking or chain extending a polymer of formula I or II.

5. An ink jet printhead according to claim 1 wherein the substituent which imparts photosensitivity to the polymer is selected from the group consisting of unsaturated ester groups, ether groups, alkylcarboxymethylene groups, epoxy groups, allyl groups, vinyl groups, unsaturated ether groups, unsaturated ammonium groups, unsaturated phosphonium groups, hydroxyalkyl groups, halomethyl groups, and mixtures thereof.

10. An ink jet printhead according to claim 1 wherein the substituent which imparts photosensitivity to the polymer is selected from the group consisting of unsaturated ester groups, halomethyl groups, and mixtures thereof.

15. An ink jet printhead according to claim 1 wherein the polymer is of Formula I.

8. An ink jet printhead according to claim 1 wherein the polymer is of Formula II.

9. An ink jet printhead according to claim 1 wherein A is



and B is



wherein z is an integer of from 2 to about 20, or a mixture thereof.

10. An ink jet printhead according to claim 1 wherein the polymer has a weight average molecular weight of from about 15,000 to about 20,000.

11. A process for forming an ink jet printhead which comprises:

(a) providing a lower substrate in which one surface 65 thereof has an array of heating elements and addressing electrodes having terminal ends formed thereon;

64

(b) depositing onto the surface of the lower substrate having the heating elements and addressing electrodes thereon a layer comprising a photopatternable polymer;

(c) exposing the layer to actinic radiation in an imagewise pattern such that the photopatternable polymer in exposed areas becomes crosslinked or chain extended and the photopatternable polymer in unexposed areas does not become crosslinked or chain extended, wherein the unexposed areas correspond to areas of the lower substrate having thereon the heating elements and the terminal ends of the addressing electrodes;

(d) removing the photopatternable polymer from the unexposed areas, thereby forming recesses in the layer, said recesses exposing the heating elements and the terminal ends of the addressing electrodes;

(e) providing an upper substrate with a set of parallel grooves for subsequent use as ink channels and a recess for subsequent use as a manifold, the grooves being open at one end for serving as droplet emitting nozzles, said upper substrate comprising a polymer of the formula



55 wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of the monomer repeat units of the polymer, A is



**65**

-continued



or mixtures thereof, B is

**66**

-continued



wherein v is an integer of from 1 to about 20,



30

wherein z is an integer of from 2 to about 20,



40 wherein u is an integer of from 1 to about 20,



65

67

wherein w is an integer of from 1 to about 20,



or mixtures thereof, and n is an integer representing the number of repeating monomer units; and

(f) aligning, mating, and bonding the upper substrate to 30 the layer of the lower substrate to form a printhead with the grooves in the upper substrate being aligned with the heating elements in the lower substrate to form droplet emitting nozzles, thereby forming a thermal ink jet printhead.

12. A process according to claim 11 wherein the photopatternable polymer is of formula I or II.

13. A process according to claim 12 wherein the resulting printhead is substantially free of an interface between the upper substrate and the layer of the lower substrate.

14. A process according to claim 11 wherein the upper substrate is bonded to the layer of the lower substrate with an adhesive which comprises a polymer of formula I or II.

15. A process according to claim 11 wherein the substituent which imparts photosensitivity to the polymer is selected from the group consisting of unsaturated ester groups, ether groups, alkylcarboxymethylene groups, epoxy groups, allyl groups, vinyl groups, unsaturated ether groups, unsaturated ammonium groups, unsaturated phosphonium groups, hydroxylalkyl groups, halomethyl groups, and mixtures thereof.

16. A process according to claim 11 wherein the substituent which imparts photosensitivity to the polymer is selected from the group consisting of unsaturated ester groups, halomethyl groups, and mixtures thereof.

68

17. A process according to claim 11 wherein the polymer is of Formula I.

18. A process according to claim 11 wherein the polymer is of Formula II.

5 19. A process according to claim 11 wherein A is



and B is



wherein z is an integer of from 2 to about 20, or a mixture thereof.

50 20. A process according to claim 11 wherein the polymer has a weight average molecular weight of from about 15,000 to about 20,000.

\* \* \* \* \*